



US009364720B2

(12) **United States Patent**  
**Mikura et al.**

(10) **Patent No.:** **US 9,364,720 B2**  
(45) **Date of Patent:** **\*Jun. 14, 2016**

(54) **GOLF BALL**

(75) Inventors: **Chiemi Mikura**, Kobe (JP); **Kazuhisa Fushihara**, Kobe (JP); **Mikio Yamada**, Kobe (JP)

(73) Assignee: **DUNLOP SPORTS CO. LTD.**, Kobe-Shi (JP)

(\*) Notice: Subject to any disclaimer, the term of this patent is extended or adjusted under 35 U.S.C. 154(b) by 510 days.

This patent is subject to a terminal disclaimer.

(21) Appl. No.: **13/339,051**

(22) Filed: **Dec. 28, 2011**

(65) **Prior Publication Data**

US 2012/0172151 A1 Jul. 5, 2012

(30) **Foreign Application Priority Data**

Dec. 29, 2010 (JP) ..... 2010-294591

(51) **Int. Cl.**

*A63B 37/06* (2006.01)  
*A63B 37/00* (2006.01)

(52) **U.S. Cl.**

CPC ..... *A63B 37/0054* (2013.01); *A63B 37/0062* (2013.01)

(58) **Field of Classification Search**

CPC ..... A63B 37/0062; A63B 37/0063  
USPC ..... 473/351, 377  
See application file for complete search history.

(56) **References Cited**

## U.S. PATENT DOCUMENTS

4,688,801 A 8/1987 Reiter  
4,726,590 A 2/1988 Molitor  
4,838,556 A 6/1989 Sullivan

4,844,471 A 7/1989 Terence et al.  
4,852,884 A 8/1989 Sullivan  
5,018,740 A 5/1991 Sullivan  
5,184,828 A 2/1993 Kim et al.  
5,403,010 A 4/1995 Yabuki et al.

(Continued)

## FOREIGN PATENT DOCUMENTS

EP 1358914 A1 11/2003  
JP 61-37178 A 2/1986

(Continued)

## OTHER PUBLICATIONS

Notice of Reasons for Rejection issued Oct. 21, 2014, in Japanese Patent Application No. 2010-294591 (English translation).

(Continued)

*Primary Examiner* — Raeann Gorden

(74) *Attorney, Agent, or Firm* — Birch, Stewart, Kolasch & Birch, LLP

(57) **ABSTRACT**

An object of the present invention is to provide a golf ball traveling a great distance of a driver shot. The present invention provides a golf ball having a spherical core and at least one cover layer covering the spherical core, wherein the spherical core is formed from a rubber composition containing (a) a base rubber, (b) an  $\alpha,\beta$ -unsaturated carboxylic acid having 3 to 8 carbon atoms and/or a metal salt thereof as a co-crosslinking agent, (c) a crosslinking initiator, (d) a carboxylic acid and/or a salt thereof, and (e) an organic sulfur compound having a naphthalene ring, provided that the rubber composition further contains (e) a metal compound in the case of containing only (b) the  $\alpha,\beta$ -unsaturated carboxylic acid having 3 to 8 carbon atoms as the co-crosslinking agent.

**19 Claims, 12 Drawing Sheets**



(56)

## References Cited

## U.S. PATENT DOCUMENTS

|                   |         |                             |                 |                |                  |
|-------------------|---------|-----------------------------|-----------------|----------------|------------------|
| 5,816,944 A       | 10/1998 | Asakura et al.              | 2010/0216905 A1 | 8/2010         | Kuwamura et al.  |
| 5,830,085 A       | 11/1998 | Higuchi et al.              | 2010/0273575 A1 | 10/2010        | Watanabe         |
| 6,056,650 A       | 5/2000  | Yamagishi et al.            | 2010/0298067 A1 | 11/2010        | Watanabe         |
| 6,258,302 B1      | 7/2001  | Nesbitt                     | 2010/0304893 A1 | 12/2010        | De Garavilla     |
| 6,277,036 B1      | 8/2001  | Hayashi et al.              | 2011/0092315 A1 | 4/2011         | Nakamura et al.  |
| 6,302,810 B2      | 10/2001 | Yokota                      | 2011/0143861 A1 | 6/2011         | Watanabe et al.  |
| 6,390,936 B1      | 5/2002  | Sugimoto                    | 2011/0143862 A1 | 6/2011         | Watanabe et al.  |
| 6,419,595 B1      | 7/2002  | Maruko et al.               | 2011/0159998 A1 | 6/2011         | Ohama et al.     |
| 6,596,797 B2      | 7/2003  | Nesbitt                     | 2011/0300968 A1 | 12/2011        | Ryu et al.       |
| 6,652,393 B1      | 11/2003 | Watanabe                    | 2012/0088604 A1 | 4/2012         | Matsuyama et al. |
| 6,666,780 B2      | 12/2003 | Watanabe                    | 2012/0172149 A1 | 7/2012         | Mikura et al.    |
| 6,705,956 B1      | 3/2004  | Moriyama et al.             | 2012/0172150 A1 | 7/2012         | Mikura et al.    |
| 6,726,579 B2      | 4/2004  | Ohama et al.                | 2012/0196699 A1 | 8/2012         | De Garavilla     |
| 6,762,247 B2      | 7/2004  | Voorheis et al.             | 2012/0329574 A1 | 12/2012        | Mikura et al.    |
| 6,815,507 B2      | 11/2004 | Ohama                       | 2012/0329575 A1 | 12/2012        | Mikura et al.    |
| 6,919,393 B2      | 7/2005  | Mano et al.                 | 2013/0005506 A1 | 1/2013         | Isogawa et al.   |
| 7,086,970 B2      | 8/2006  | Hayashi et al.              | 2013/0005507 A1 | 1/2013         | Sajima et al.    |
| 7,300,363 B2      | 11/2007 | Kasashima                   | 2013/0005508 A1 | 1/2013         | Matsuyama et al. |
| 7,329,194 B2      | 2/2008  | Watanabe et al.             | 2013/0017905 A1 | 1/2013         | Shindo et al.    |
| 7,344,455 B1      | 3/2008  | Higuchi                     | 2013/0053182 A1 | 2/2013         | Tarao et al.     |
| 7,682,266 B2      | 3/2010  | Endo et al.                 | 2013/0065707 A1 | 3/2013         | Matsuyama        |
| 7,914,397 B2      | 3/2011  | Endo et al.                 | 2013/0123044 A1 | 5/2013         | Mikura et al.    |
| 8,044,164 B2      | 10/2011 | Shiga et al.                | 2013/0123045 A1 | 5/2013         | Watanabe et al.  |
| 8,393,978 B2      | 3/2013  | Watanabe et al.             | 2013/0172111 A1 | 7/2013         | Sakamine et al.  |
| 8,523,707 B2      | 9/2013  | Watanabe et al.             | 2013/0244810 A1 | 9/2013         | Mikura et al.    |
| 8,722,752 B2      | 5/2014  | Kuwamura et al.             | 2013/0288824 A1 | 10/2013        | Isogawa et al.   |
| 8,777,780 B2      | 7/2014  | Kamino et al.               | 2013/0303307 A1 | 11/2013        | Sakamine et al.  |
| 2001/0026027 A1   | 10/2001 | Nesbitt                     | 2013/0310196 A1 | 11/2013        | Okabe            |
| 2001/0034412 A1   | 10/2001 | Nesbitt                     | 2013/0316850 A1 | 11/2013        | Inoue et al.     |
| 2002/0032077 A1   | 3/2002  | Watanabe                    | 2013/0324631 A1 | 12/2013        | Kuwamura et al.  |
| 2002/0052254 A1   | 5/2002  | Ichikawa et al.             |                 |                |                  |
| 2002/0155905 A1   | 10/2002 | Iwami                       | JP              | 61-113475 A    | 5/1986           |
| 2002/0187856 A1   | 12/2002 | Endou                       | JP              | 61-253079 A    | 11/1986          |
| 2003/0114249 A1   | 6/2003  | Voorheis et al.             | JP              | 61-258844 A    | 11/1986          |
| 2003/0114252 A1   | 6/2003  | Hayashi et al.              | JP              | 62-14870 A     | 1/1987           |
| 2003/0119606 A1   | 6/2003  | Ohama et al.                | JP              | 62-82981 A     | 4/1987           |
| 2003/0134946 A1   | 7/2003  | Kataoka                     | JP              | 6-154357 A     | 6/1994           |
| 2003/0144425 A1   | 7/2003  | Mano et al.                 | JP              | 8-322964 A     | 12/1996          |
| 2003/0171165 A1   | 9/2003  | Watanabe                    | JP              | 9-313643 A     | 12/1997          |
| 2003/0207999 A1 * | 11/2003 | Higuchi et al. .... 525/274 | JP              | 11-9720 A      | 1/1999           |
| 2003/0208000 A1   | 11/2003 | Higuchi et al.              | JP              | 11-47309 A     | 2/1999           |
| 2003/0216193 A1 * | 11/2003 | Graves et al. .... 473/351  | JP              | 2000-60999 A   | 2/2000           |
| 2004/0106475 A1   | 6/2004  | Sasaki et al.               | JP              | 2000-84118 A   | 3/2000           |
| 2004/0110906 A1   | 6/2004  | Fujisawa et al.             | JP              | 2000-245873 A  | 9/2000           |
| 2005/0137031 A1   | 6/2005  | Kataoka et al.              | JP              | 2000-271248 A  | 10/2000          |
| 2005/0187353 A1   | 8/2005  | Goguen et al.               | JP              | 2001-17569 A   | 1/2001           |
| 2006/0019771 A1   | 1/2006  | Kennedy, III et al.         | JP              | 2002-764 A     | 1/2001           |
| 2006/0025238 A1   | 2/2006  | Endo et al.                 | JP              | 2002-540821 A  | 12/2002          |
| 2006/0128900 A1 * | 6/2006  | Nanba et al. .... 525/261   | JP              | 2003-135627 A  | 5/2003           |
| 2006/0135287 A1   | 6/2006  | Kennedy, III et al.         | JP              | 2003-164546 A  | 6/2003           |
| 2006/0178231 A1   | 8/2006  | Kasashima                   | JP              | 2003-180872 A  | 7/2003           |
| 2007/0129174 A1   | 6/2007  | Higuchi                     | JP              | 2003-226782 A  | 8/2003           |
| 2007/0173607 A1   | 7/2007  | Kennedy et al.              | JP              | 2003-320054 A  | 11/2003          |
| 2007/0281801 A1   | 12/2007 | Watanabe et al.             | JP              | 2003-320055 A  | 11/2003          |
| 2007/0281802 A1   | 12/2007 | Watanabe et al.             | JP              | 2003-325703 A  | 11/2003          |
| 2008/0020863 A1   | 1/2008  | Higuchi et al.              | JP              | 2004-73856 A   | 3/2004           |
| 2008/0020864 A1   | 1/2008  | Shindo et al.               | JP              | 2004-167052 A  | 6/2004           |
| 2008/0076603 A1   | 3/2008  | Shindo et al.               | JP              | 2005-179522 A  | 7/2005           |
| 2008/0161134 A1   | 7/2008  | Tarao                       | JP              | 2006-34740 A   | 2/2006           |
| 2008/0194357 A1   | 8/2008  | Higuchi                     | JP              | 2006-218294 A  | 8/2006           |
| 2008/0194358 A1   | 8/2008  | Higuchi                     | JP              | 2006-297108 A  | 11/2006          |
| 2008/0194359 A1   | 8/2008  | Higuchi et al.              | JP              | 2007-152090 A  | 6/2007           |
| 2008/0214324 A1   | 9/2008  | Nanba et al.                | JP              | 2007-319660 A  | 12/2007          |
| 2008/0214325 A1   | 9/2008  | Higuchi et al.              | JP              | 2008-523952 A  | 7/2008           |
| 2008/0274835 A1   | 11/2008 | Comeau et al.               | JP              | 2008-194471 A  | 8/2008           |
| 2008/0305890 A1   | 12/2008 | Watanabe et al.             | JP              | 2008-194473 A1 | 8/2008           |
| 2008/0312008 A1   | 12/2008 | Higuchi et al.              | JP              | 2008-212681 A  | 9/2008           |
| 2009/0105013 A1   | 4/2009  | Slagel et al.               | JP              | 2009-11431 A   | 1/2009           |
| 2009/0111611 A1   | 4/2009  | Kimura et al.               | JP              | 2009-11436 A   | 1/2009           |
| 2009/0124757 A1   | 5/2009  | Shindo et al.               | JP              | 2009-119256 A  | 6/2009           |
| 2009/0143169 A1   | 6/2009  | Shiga et al.                | JP              | 2009-131508 A  | 6/2009           |
| 2009/0227394 A1   | 9/2009  | Bulpett et al.              | JP              | 2010-68997 A   | 4/2010           |
| 2010/0009776 A1   | 1/2010  | Okabe et al.                | JP              | 2010-162323 A  | 7/2010           |
| 2010/0069175 A1   | 3/2010  | Kamino et al.               | JP              | 2010-253268 A  | 11/2010          |
| 2010/0137076 A1   | 6/2010  | Endo et al.                 | JP              | 2011-83395 A   | 4/2011           |
|                   |         |                             | JP              | 2011-120898 A  | 6/2011           |

## FOREIGN PATENT DOCUMENTS

(56)

**References Cited**

## FOREIGN PATENT DOCUMENTS

JP 2011-255172 A 12/2011  
KR 10-0995019 B1 11/2010  
WO WO 2009/051114 A1 4/2009

## OTHER PUBLICATIONS

Chinese Office Action, dated Dec. 16, 2013, for Chinese Application No. 201110411055.8.  
Chinese Office Action, dated Dec. 27, 2013, for Chinese Application No. 201110411053.9.  
Chinese Office Action, dated Dec. 27, 2013, for Chinese Application No. 201110463019.6.  
Chinese Office Action, dated Dec. 27, 2013, for Chinese Application No. 201110463020.9.  
Chinese Office Action, dated Jan. 24, 2014, for Chinese Application No. 201110411896.9.  
Chinese Office Action, dated Nov. 29, 2013, for Chinese Application No. 201110411898.8.  
Dupont, Hardness Conversion, uploaded Jun. 12, 2014, Dupont, 1 page.  
European Office Action, dated Mar. 4, 2014, for European Application No. 12172672.3.  
Examiner's Calc, JIS-C hardness converted by Dupont cited in the U.S. Office Action, dated May 30, 2014, for U.S. Appl. No. 13/494,315.  
Extended European Search Report, dated Dec. 19, 2013, for European Application No. 12199433.9.  
Extended European Search Report, dated Mar. 5, 2013, for European Application No. 12172666.5.  
Extended European Search Report, dated Mar. 5, 2013, for European Application No. 12172672.3.  
Japanese Notice of Reasons for Rejection, dated Oct. 15, 2013, for Japanese Application No. 2011-139901 (English translation only provided).

Japanese Notice of Reasons for Rejection, dated Oct. 15, 2013, for Japanese Application No. 2011-164724 (English translation only provided).

Japanese Notice of Reasons for Rejection, dated Oct. 15, 2013, for Japanese Application No. 2011-164725 (English translation only provided).

Japanese Notice of Reasons for Rejection, dated Oct. 15, 2013, for Japanese Application No. 2012-116655 (English translation only provided).

Korean Office Action, dated Jul. 16, 2013, for Korean Application No. 10-2012-0060983.

Korean Office Action, dated Jul. 16, 2013, for Korean Application No. 10-2012-0060985.

Korean Office Action, dated Oct. 17, 2013, for Korean Application No. 10-2012-0127170.

U.S. Office Action, dated Apr. 24, 2014, for U.S. Appl. No. 13/599,441.

U.S. Office Action, dated Feb. 10, 2014, for U.S. Appl. No. 13/309,965.

U.S. Office Action, dated Feb. 6, 2014, for U.S. Appl. No. 13/337,607.

U.S. Office Action, dated Jul. 25, 2014, for U.S. Appl. No. 13/545,658.

U.S. Office Action, dated May 21, 2014, for U.S. Appl. No. 13/309,965.

U.S. Office Action, dated May 22, 2014, for U.S. Appl. No. 13/337,607.

U.S. Office Action, dated May 29, 2014, for U.S. Appl. No. 13/606,378.

U.S. Office Action, dated May 30, 2014, for U.S. Appl. No. 13/494,315.

U.S. Office Action, dated May 8, 2014, for U.S. Appl. No. 13/338,868.

\* cited by examiner



Fig. 1

**Fig. 2**



Fig. 3



Fig. 4



Fig. 5



Fig. 6



Fig. 7



Fig. 8



Fig. 9



Fig. 10



Fig. 11



Fig. 12

**1**  
**GOLF BALL**

**FIELD OF THE INVENTION**

The present invention relates to a golf ball excellent in flying performance, in particular, an improvement of a core of a golf ball.

**DESCRIPTION OF THE RELATED ART**

As a method for improving a flight distance on driver shots, for example, there are methods of using a core having high resilience and using a core having a hardness distribution in which the hardness increases toward the surface of the core from the center thereof. The former method has an effect of enhancing an initial speed, and the latter method has an effect of a higher launch angle and a lower spin rate. A golf ball having a higher launch angle and a lower spin rate travels a great distance.

For example, Japanese Patent Publications Nos. S61-37178 A, 2008-212681 A, 2008-523952 A and 2009-119256 A disclose a technique of enhancing resilience of the core. Japanese Patent Publication No. 61-37178 A discloses a solid golf ball having a PGA ball compression from 80 to 95. The solid golf ball has an inner core where 5 wt % to 25 wt % of palmitic acid, stearic acid, or myristic acid as a co-crosslinking activator, 20 wt % or more of zinc oxide as another co-crosslinking activator, 1 wt % to 3 wt % of a reaction rate retarder are blended with respect to zinc acrylate when blending 25 parts to 45 parts by weight of zinc acrylate as a co-crosslinking agent to 100 parts by weight of the rubber.

Japanese Patent Publication No. 2008-212681 A discloses a golf ball comprising, as a component, a molded and crosslinked product obtained from a rubber composition essentially comprising a base rubber, a filler, an organic peroxide, an  $\alpha,\beta$ -unsaturated carboxylic acid and/or a metal salt thereof, a copper salt of a saturated or unsaturated fatty acid.

Japanese Patent Publication No. 2008-523952 T discloses a golf ball, or a component thereof, molded from a composition comprising a base elastomer selected from the group consisting of polybutadiene and mixtures of polybutadiene with other elastomers, at least one metallic salt of an unsaturated monocarboxylic acid, a free radical initiator, and a non-conjugated diene monomer.

Japanese Patent Publication No. 2009-119256 A discloses a method of manufacturing a golf ball, comprising preparing a masterbatch of an unsaturated carboxylic acid and/or a metal salt thereof by mixing the unsaturated carboxylic acid and/or the metal salt thereof with a rubber material ahead, using the masterbatch to prepare a rubber composition containing the rubber material, and employing a heated and molded product of the rubber composition as a golf ball component, wherein the masterbatch of the unsaturated carboxylic acid and/or the metal salt thereof comprises; (A) from 20 wt % to 100 wt % of a modified polybutadiene obtained by modifying a polybutadiene having a vinyl content of from 0 to 2%, a cis-1,4 bond content of at least 80% and active terminals, the active terminal being modified with at least one type of alkoxysilane compound, and (B) from 80 wt % to 0 wt % of a diene rubber other than (A) the above rubber component [the figures are represented by wt % in the case that a total amount of (A) and (B) equals to 100 wt %] and (C) an unsaturated carboxylic acid and/or a metal salt thereof.

For example, Japanese Patent Publications Nos. H6-154357 A, 2008-194471 A, 2008-194473 A and 2010-253268 A disclose a core having a hardness distribution.

**2**

Japanese Patent Publication No. H6-154357 A discloses a two-piece golf ball comprising a core formed of a rubber composition containing a base rubber, a co-crosslinking agent, and an organic peroxide, and a cover covering said core, wherein the core has the following hardness distribution according to JIS-C type hardness meter readings: (1) hardness at center: 58-73, (2) hardness at 5 to 10 mm from center: 65-75, (3) hardness at 15 mm from center: 74-82, (4) surface hardness: 76-84, wherein hardness (2) is almost constant within the above range, and the relation (1)<(2)<(3)<(4) is satisfied.

Japanese Patent Publication No. 2008-194471 A discloses a solid golf ball comprising a solid core and a cover layer that encases the core, wherein the solid core is formed of a rubber composition composed of 100 parts by weight of a base rubber that includes from 60 to 100 parts by weight of a polybutadiene rubber having a cis-1,4 bond content of at least 60% and synthesized using a rare-earth catalyst, from 0.1 to 5 parts by weight of an organic sulfur compound, an unsaturated carboxylic acid or a metal salt thereof, an inorganic filler, and an antioxidant; the solid core has a deformation from 2.0 mm to 4.0 mm, when applying a load from an initial load of 10 kgf to a final load of 130 kgf and has the hardness distribution shown in the following table.

TABLE 1

| Hardness distribution in solid core            | Shore D harness |
|------------------------------------------------|-----------------|
| Center                                         | 30 to 48        |
| Region located 4 mm from center                | 34 to 52        |
| Region located 8 mm from center                | 40 to 58        |
| Region located 12 mm from center (Q)           | 43 to 61        |
| Region located 2 to 3 mm inside of surface (R) | 36 to 54        |
| Surface (S)                                    | 41 to 59        |
| Hardness difference [(Q) - (S)]                | 1 to 10         |
| Hardness difference [(S) - (R)]                | 3 to 10         |

Japanese Patent Publication No. 2008-194473 A discloses a solid golf ball comprising a solid core and a cover layer that encases the core, wherein the solid core is formed of a rubber composition composed of 100 parts by weight of a base rubber that includes from 60 to 100 parts by weight of a polybutadiene rubber having a cis-1,4 bond content of at least 60% and synthesized using a rare-earth catalyst, from 0.1 to 5 parts by weight of an organic sulfur compound, an unsaturated carboxylic acid or a metal salt thereof, and an inorganic filler; the solid core has a deformation from 2.0 mm to 4.0 mm, when applying a load from an initial load of 10 kgf to a final load of 130 kgf and has the hardness distribution shown in the following table.

TABLE 2

| Hardness distribution in solid core            | Shore D harness |
|------------------------------------------------|-----------------|
| Center                                         | 25 to 45        |
| Region located 5 to 10 mm from center          | 39 to 58        |
| Region located 15 mm from center               | 36 to 55        |
| Surface (S)                                    | 55 to 75        |
| Hardness difference between center and surface | 20 to 50        |

Japanese Patent Publication No. 2010-253268 A discloses a multi-piece solid golf ball comprising a core, an envelope layer encasing the core, an intermediate layer encasing the envelope layer, and a cover which encases the intermediate layer and has formed on a surface thereof a plurality of dimples, wherein the core is formed primarily of a rubber material and has a hardness which gradually increases from a

center to a surface thereof, the hardness difference in JIS-C hardness units between the core center and the core surface being at least 15 and, letting (I) be the average value for cross-sectional hardness at a position about 15 mm from the core center and at the core center and letting (II) be the cross-sectional hardness at a position about 7.5 mm from the core center, the hardness difference (I)-(II) in JIS-C units being within  $\pm 2$ ; and the envelope layer, intermediate layer and cover have hardness which satisfy the condition: cover hardness > intermediate layer hardness > envelope layer hardness.

### SUMMARY OF THE INVENTION

An object of the present invention is to provide a golf ball 15 traveling a great flight distance on driver shots.

The present invention provides a golf ball comprising a spherical core and at least one cover layer covering the spherical core, wherein the spherical core is formed from a rubber composition containing (a) a base rubber, (b) an unsaturated carboxylic acid having 3 to 8 carbon atoms and/or a metal salt thereof as a co-crosslinking agent, (c) a crosslinking initiator, and (d) a carboxylic acid and/or a salt thereof, and (e) an organic sulfur compound having a naphthalene ring, provided that the rubber composition further contains (f) a metal compound in the case of containing only (b) the  $\alpha,\beta$ -unsaturated carboxylic acid having 3 to 8 carbon atoms as the co-crosslinking agent.

The present invention is configured as described above and a gist of the present invention resides in that the spherical core has a hardness distribution where the hardness increases linearly or almost linearly from the center of the core toward the surface thereof. The spherical core having the hardness distribution where the hardness increases linearly or almost linearly from the center of the core toward the surface thereof, with a high degree of the outer-hard and inner-soft structure reduces the spin rate on driver shots, thereby providing a greater flight distance on driver shots. Furthermore, the resilience of the core enhances, since (e) the organic sulfur compound having the naphthalene ring is used as an essential component in the present invention. As a result of these synergic actions, the golf ball of the present invention travels a great flight distance on driver shots. In general, if the degree of the outer-hard and inner-soft structure of the core increases, the resilience lowers. However, in the present invention, use of (d) the carboxylic acid and/or the salt thereof and (e) the organic sulfur compound having the naphthalene ring in combination further improves the resilience of the core, as well as allows the core to have the hardness distribution where the hardness increases linearly or almost linearly, with the high degree of the outer-hard and inner-soft structure.

The reason why the spherical core formed from the rubber composition has the hardness distribution where the hardness increases linearly or almost linearly from the center of the core toward the surface thereof is considered as follows. When molding the core, the internal temperature of the core is high at the core central part and decreases toward the core surface, since reaction heat from a crosslinking reaction of the base rubber accumulates at the core central part. (d) The carboxylic acid and/or a salt thereof reacts with the metal salt of (b) the  $\alpha,\beta$ -unsaturated carboxylic acid having 3 to 8 carbon atoms, when molding the core. That is, (d) the carboxylic acid and/or the salt thereof exchanges a cation with the metal salt of the  $\alpha,\beta$ -unsaturated carboxylic acid having 3 to 8 carbon atoms, thereby breaking the metal crosslinking by the metal salt of the  $\alpha,\beta$ -unsaturated carboxylic acid having 3

to 8 carbon atoms. This cation exchange reaction easily occurs at the core central part where the temperature is high, and less occurs toward the core surface. In other words, the breaking of the metal crosslinking easily occurs at the core central part, but less occurs toward the surface. As a result, it is conceivable that since a crosslinking density in the core increases from the center of the core toward the surface thereof, the core hardness increases linearly or almost linearly from the center of the core toward the surface thereof. In the present invention, by using (e) the organic sulfur compound having the naphthalene ring and (d) the carboxylic acid and/or the salt thereof in combination, the degree of the outer-hard and inner-soft structure of the core can be further enhanced.

According to the present invention, it is possible to provide a golf ball traveling a great flight distance on driver shots.

### BRIEF DESCRIPTION OF THE DRAWINGS

FIG. 1 is a graph showing the hardness distribution of the spherical core;

FIG. 2 is a graph showing the hardness distribution of the spherical core;

FIG. 3 is a graph showing the hardness distribution of the spherical core;

FIG. 4 is a graph showing the hardness distribution of the spherical core;

FIG. 5 is a graph showing the hardness distribution of the spherical core;

FIG. 6 is a graph showing the hardness distribution of the spherical core;

FIG. 7 is a graph showing the hardness distribution of the spherical core;

FIG. 8 is a graph showing the hardness distribution of the spherical core;

FIG. 9 is a graph showing the hardness distribution of the spherical core;

FIG. 10 is a graph showing the hardness distribution of the spherical core;

FIG. 11 is a graph showing the hardness distribution of the spherical core; and

FIG. 12 is a graph showing the hardness distribution of the spherical core.

### DESCRIPTION OF THE PREFERRED EMBODIMENT

The present invention provides a golf ball comprising a spherical core and at least one cover layer, wherein the spherical core is formed from a rubber composition containing (a) a base rubber, (b) an  $\alpha,\beta$ -unsaturated carboxylic acid having 3 to 8 carbon atoms and/or a metal salt thereof as a co-crosslinking agent, (c) an co-crosslinking initiator, and (d) a carboxylic acid and/or a salt thereof, and (e) an organic sulfur compound having a naphthalene ring, provided that the rubber composition further contains (f) a metal compound in the case of containing only (b) the  $\alpha,\beta$ -unsaturated carboxylic acid having 3 to 8 carbon atoms as the co-crosslinking initiator.

First, (a) the base rubber used in the present invention will be explained. As (a) the base rubber used in the present invention, natural rubber and/or synthetic rubber can be used. For example, polybutadiene rubber, natural rubber, polyisoprene rubber, styrene polybutadiene rubber, ethylene-propylene-diene rubber (EPDM), or the like can be used. These rubbers may be used solely or two or more of these rubbers may be used in combination. Among them, typically preferred is the high cis-polybutadiene having a cis-1,4 bond in

a proportion of 40% or more, more preferably 80% or more, even more preferably 90% or more in view of its superior resilience property.

The high-cis polybutadiene preferably has a 1,2-vinyl bond in a content of 2 mass % or less, more preferably 1.7 mass % or less, and even more preferably 1.5 mass % or less. If the content of 1,2-vinyl bond is excessively high, the resilience may be lowered.

The high-cis polybutadiene is preferably one synthesized using a rare earth element catalyst. When a neodymium catalyst, which employs a neodymium compound which is a lanthanum series rare earth element compound, is used, a polybutadiene rubber having a high content of a cis-1,4 bond and a low content of a 1,2-vinyl bond is obtained with excellent polymerization activity. Such a polybutadiene rubber is particularly preferred.

The high-cis polybutadiene preferably has a Mooney viscosity (ML<sub>1+4</sub> (100° C.)) of 30 or more, more preferably 32 or more, even more preferably 35 or more, and preferably has a Mooney viscosity (ML<sub>1+4</sub> (100° C.)) of 140 or less, more preferably 120 or less, even more preferably 100 or less, and most preferably 80 or less. It is noted that the Mooney viscosity (ML<sub>1+4</sub> (100° C.)) in the present invention is a value measured according to JIS K6300 using an L rotor under the conditions of: a preheating time of 1 minute; a rotor revolution time of 4 minutes; and a temperature of 100° C.

The high-cis polybutadiene preferably has a molecular weight distribution Mw/Mn (Mw: weight average molecular weight, Mn: number average molecular weight) of 2.0 or more, more preferably 2.2 or more, even more preferably 2.4 or more, and most preferably 2.6 or more, and preferably has a molecular weight distribution Mw/Mn of 6.0 or less, more preferably 5.0 or less, even more preferably 4.0 or less, and most preferably 3.4 or less. If the molecular weight distribution (Mw/Mn) of the high-cis polybutadiene is excessively low, the processability may deteriorate. If the molecular weight distribution (Mw/Mn) of the high-cis polybutadiene is excessively high, the resilience may be lowered. It is noted that the measurement of the molecular weight distribution is conducted by gel permeation chromatography ("HLC-8120GPC", manufactured by Tosoh Corporation) using a differential refractometer as a detector under the conditions of column: GMHHXL (manufactured by Tosoh Corporation), column temperature: 40° C., and mobile phase: tetrahydrofuran, and calculated by converting based on polystyrene standard.

Next, (b) the α,β-unsaturated carboxylic acid having 3 to 8 carbon atoms and/or a metal salt thereof will be explained. (b) The α,β-unsaturated carboxylic acid having 3 to 8 carbon atoms and/or a metal salt thereof is blended as a co-crosslinking agent in the rubber composition and has an action of crosslinking a rubber molecule by graft polymerization to a base rubber molecular chain. In the case that the rubber composition used in the present invention contains only the α,β-unsaturated carboxylic acid having 3 to 8 carbon atoms as the co-crosslinking agent, the rubber composition preferably further contains (f) a metal compound. Neutralizing the α,β-unsaturated carboxylic acid having 3 to 8 carbon atoms with the metal compound in the rubber composition provides substantially the same effect as using the metal salt of the α,β-unsaturated carboxylic acid having 3 to 8 carbon atoms. Further, in the case of using the α,β-unsaturated carboxylic acid having 3 to 8 carbon atoms and the metal salt thereof in combination, (f) the metal compound may be used.

The α,β-unsaturated carboxylic acid having 3 to 8 carbon atoms includes, for example, acrylic acid, methacrylic acid, fumaric acid, maleic acid, crotonic acid, and the like.

Examples of the metals constituting the metal salts of the α,β-unsaturated carboxylic acid having 3 to 8 carbon atoms include: monovalent metal ions such as sodium, potassium, lithium or the like; divalent metal ions such as magnesium, calcium, zinc, barium, cadmium or the like; trivalent metal ions such as aluminum ion or the like; and other metal ions such as tin, zirconium or the like. The above metal ions can be used solely or as a mixture of at least two of them. Among these metal ions, divalent metal ions such as magnesium, calcium, zinc, barium, cadmium or the like are preferable. Use of the divalent metal salts of the α,β-unsaturated carboxylic acid having 3 to 8 carbon atoms easily generates a metal crosslinking between the rubber molecules. Especially, as the divalent metal salt, zinc acrylate is preferable, because zinc acrylate enhances the resilience of the resultant golf ball. The α,β-unsaturated carboxylic acid having 3 to 8 carbon atoms and/or a metal salt thereof may be used solely or in combination at least two of them.

The content of (b) the α,β-unsaturated carboxylic acid having 3 to 8 carbon atoms and/or the metal salt thereof is preferably 15 parts by mass or more, more preferably 20 parts by mass or more, and is preferably 50 parts by mass or less, more preferably 45 parts by mass or less, even more preferably 35 parts by mass or less, with respect to 100 parts by mass of (a) the base rubber. If the content of (b) the α,β-unsaturated carboxylic acid having 3 to 8 carbon atoms and/or the metal salt thereof is less than 15 parts by mass, the content of (c) the co-crosslinking initiator which will be explained below must be increased in order to obtain the appropriate hardness of the constituting member formed from the rubber composition, which tends to cause the lower resilience. On the other hand, if the content of (b) the α,β-unsaturated carboxylic acid having 3 to 8 carbon atoms and/or the metal salt thereof exceeds 50 parts by mass, the constituting member formed from the rubber composition becomes excessively hard, which tends to cause the lower shot feeling.

(c) The crosslinking initiator is blended in order to crosslink (a) the base rubber component. As (c) the crosslinking initiator, an organic peroxide is preferred. Specific examples of the organic peroxide include organic peroxides such as dicumyl peroxide, 1,1-bis(t-butylperoxy)-3,3,5-trimethylcyclohexane, 2,5-dimethyl-2,5-di(t-butylperoxy)hexane, and di-t-butyl peroxide. These organic peroxides may be used solely or two or more of these organic peroxides may be used in combination. Among them, dicumyl peroxide is preferably used.

The content of (c) the crosslinking initiator is preferably 0.2 part by mass or more, and more preferably 0.5 part by mass or more, and is preferably 5.0 parts by mass or less, and more preferably 2.5 parts by mass or less, with respect to 100 parts by mass of (a) the base rubber. If the content of (c) the crosslinking initiator is less than 0.2 part by mass, the constituting member formed from the rubber composition becomes too soft, and thus the golf ball may have the lower resilience. If the content of (c) the crosslinking initiator exceeds 5.0 parts by mass, the amount of (b) the co-crosslinking agent must be decreased in order to obtain the appropriate hardness of the constituting member formed from the rubber composition, resulting in the insufficient resilience and lower durability of the golf ball.

(d) The carboxylic acid and/or a salt thereof used in the present invention will be explained. It is considered that (d) the carboxylic acid and/or the salt thereof has an action of breaking the metal crosslinking by the metal salt of the α,β-unsaturated carboxylic acid having 3 to 8 carbon atoms at the center part of the core, when molding the core. Although (d) the carboxylic acid and/or the salt thereof used in the present

invention is not limited as long as it is a compound having a carboxyl group, (b) the  $\alpha,\beta$ -unsaturated carboxylic acid having 3 to 8 carbon atoms used as a co-crosslinking agent should not be included.

(d) The carboxylic acid may include any one of an aliphatic carboxylic acid (sometimes may be merely referred to as "fatty acid" in the present invention) and an aromatic carboxylic acid, as long as it exchanges the cation component with the metal salt of the  $\alpha,\beta$ -unsaturated carboxylic acid having 3 to 8 carbon atoms. The carboxylic acid preferably includes a carboxylic acid having 4 to 30 carbon atoms, more preferably a carboxylic acid having 9 to 30 carbon atoms, even more preferably a carboxylic acid having 14 to 28 carbon atoms.

The fatty acid may be either a saturated fatty acid or an unsaturated fatty acid; however, a saturated fatty acid is preferable. Specific examples of the saturated fatty acids are butyric acid (C4), valeric acid (C5), caproic acid (C6), enanthic acid (C7), caprylic acid (C8), pelargonic acid (C9), capric acid (C10), lauric acid (C12), myristic acid (C14), myristoleic acid (C14), pentadecylic acid (C15), palmitic acid (C16), palmitoleic acid (C16), margaric acid (C17), stearic acid (C18), elaidic acid (C18), vaccenic acid (C18), oleic acid (C18), linoleic acid (C18), linolenic acid (C18), 12-hydroxystearic acid (C18), arachidic acid (C20), gadoleic acid (C20), arachidonic acid (C20), eicosenoic acid (C20), behenic acid (C22), erucic acid (C22), lignoceric acid (C24), nervonic acid (C24), cerotic acid (C26), montanic acid (C28), and melissic acid (C30). The fatty acid may be used alone or as a mixture of at least two of them. Among those described above, myristic acid, palmitic acid, setaric acid, behenic acid and oleic acid are preferable as the fatty acid.

There is no particular limitation on the aromatic carboxylic acid as long as it is a compound that has an aromatic ring and a carboxyl group. Specific examples of the aromatic carboxylic acid include, for example, benzoic acid, phthalic acid, isophthalic acid, terephthalic acid, hemimellitic acid (benzene-1,2,3-tricarboxylic acid), trimellitic acid (benzene-1,2,4-tricarboxylic acid), trimesic acid (benzene-1,3,5-tricarboxylic acid), mellophanic acid (benzene-1,2,3,4-tetracarboxylic acid), prehnitic acid (benzene-1,2,3,5-tetracarboxylic acid), pyromellitic acid (benzene-1,2,4,5-tetracarboxylic acid), mellitic acid (benzene hexacarboxylic acid), diphenic acid (biphenyl-2,2'-dicarboxylic acid), toluic acid (methylbenzoic acid), xylic acid, prehnitylic acid (2,3,4-trimethylbenzoic acid),  $\gamma$ -isodurylic acid (2,3,5-trimethylbenzoic acid), durylic acid (2,4,5-trimethylbenzoic acid),  $\beta$ -isodurylic acid (2,4,6-trimethylbenzoic acid),  $\alpha$ -isodurylic acid (3,4,5-trimethylbenzoic acid), cumin acid (4-isopropylbenzoic acid), uvitic acid (5-methylisophthalic acid),  $\alpha$ -toluic acid (phenylacetic acid), hydratropic acid (2-phenylpropanoic acid), and hydrocinnamic acid (3-phenylpropanoic acid).

Furthermore, the aromatic carboxylic acid including a substitution with hydroxyl group, alkoxy group, or oxo group includes, for example, salicylic acid (2-hydroxybenzoic acid), anisic acid (methoxybenzoic acid), cresotinic acid (hydroxy(methyl)benzoic acid), o-homosalicylic acid (2-hydroxy-3-methylbenzoic acid), m-homosalicylic acid (2-hydroxy-4-methylbenzoic acid), p-homosalicylic acid (2-hydroxy-5-methylbenzoic acid), o-pyrocatechic acid (2,3-dihydroxybenzoic acid),  $\beta$ -resorcylic acid (2,4-dihydroxybenzoic acid),  $\gamma$ -resorcylic acid (2,6-dihydroxybenzoic acid), protocatechic acid (3,4-dihydroxybenzoic acid),  $\alpha$ -resorcylic acid (3,5-dihydroxybenzoic acid), vanillic acid (4-hydroxy-3-methoxybenzoic acid), isovanillic acid (3-hydroxy-4-methoxybenzoic acid), veratric acid (3,4-

dimethoxybenzoic acid), o-veratric acid (2,3-dimethoxybenzoic acid), orsellinic acid (2,4-dihydroxy-6-methylbenzoic acid), m-hemipic acid (4,5-dimethoxyphthalic acid), gallic acid (3,4,5-trihydroxybenzoic acid), syringic acid (4-hydroxy-3,5-dimethoxybenzoic acid), asaronic acid (2,4,5-trimethoxybenzoic acid), mandelic acid (hydroxy(phenyl)acetic acid), vanillylmandelic acid (hydroxy(4-hydroxy-3-methoxy phenyl)acetic acid), homoanisic acid ((4-methoxy phenyl)acetic acid), homogenitoxic acid ((2,5-dihydroxyphenyl)acetic acid), homoprotocatechic acid ((3,4-dihydroxyphenyl)acetic acid), homovanillic acid ((4-hydroxy-3-methoxy phenyl)acetic acid), homoisovanillic acid ((3-hydroxy-4-methoxy phenyl)acetic acid), homoveratric acid ((3,4-dimethoxy phenyl)acetic acid), o-homoveratric acid ((2,3-dimethoxy phenyl)acetic acid), homophthalic acid (2-(carboxymethyl)benzoic acid), homoisophthalic acid (3-(carboxymethyl)benzoic acid), homoterephthalic acid (4-(carboxymethyl)benzoic acid), phthalonic acid (2-(carboxycarbonyl)benzoic acid), isophthalonic acid (3-(carboxycarbonyl)benzoic acid), terephthalonic acid (4-(carboxycarbonyl)benzoic acid), benzilic acid (hydroxy diphenylacetic acid), atrolactic acid (2-hydroxy-2-phenylpropanoic acid), tropic acid (3-hydroxy-2-phenylpropanoic acid), melilotic acid (3-(2-hydroxyphenyl)propanoic acid), phloretic acid (3-(4-hydroxy phenyl)propanoic acid), hydrocaffic acid (3-(3,4-dihydroxyphenyl)proparluic acid), hydroferulic acid (3-(4-hydroxy-3-methoxy phenyl)propanoic acid), hydroisoferulic acid (3-(3-hydroxy-4-methoxy phenyl)propanoic acid), p-coumaric acid (3-(4-hydroxy phenyl)acrylic acid), umbellic acid (3-(2,4-dihydroxyphenyl)acrylic acid), caffeic acid (3-(3,4-dihydroxyphenyl)acrylic acid), ferulic acid (3-(4-hydroxy-3-methoxy phenyl)acrylic acid), isoferulic acid (3-(3-hydroxy-4-methoxy phenyl)acrylic acid), and sinapic acid (3-(4-hydroxy-3,5-dimethoxy phenyl)acrylic acid).

As (d) the salt of the carboxylic acid, a salt of the above described carboxylic acid may be used. A cation component of the salt of the carboxylic acid may be any one of a metal ion, an ammonium ion and an organic cation.

The metal ion includes, for example: monovalent metal ions of sodium, potassium, lithium, silver, and the like; bivalent metal ions of magnesium, calcium, zinc, barium, cadmium, copper, cobalt, nickel, manganese, and the like; trivalent metal ions of aluminum, iron, and the like; and other ions of tin, zirconium, titanium, and the like. The cation component may be used solely or as a mixture of two or more of them.

The organic cation is a cation that has a carbon chain. The organic cation includes, for example, without limitation, an organic ammonium ion. The organic ammonium ion includes, for example: primary ammonium ions such as stearyl ammonium ion, hexyl ammonium ion, octyl ammonium ion, and 2-ethyl hexyl ammonium ion; secondary ammonium ions such as dodecyl(lauryl) ammonium ion and octadecyl(stearyl) ammonium ion; tertiary ammonium ions such as trioctyl ammonium ion; and quaternary ammonium ions such as dioctyldimethyl ammonium ion and distearyldimethyl ammonium ion. The organic cation component may be used solely or as a mixture of two or more of them.

As (d) the salt of the carboxylic acid, more preferred is the potassium salt, magnesium salt, aluminum salt, zinc salt, iron salt, copper salt, nickel salt, or cobalt salt of myristic acid, palmitic acid, stearic acid, behenic acid, and oleic acid.

The content of (d) the carboxylic acid and/or the salt thereof is preferably 5 parts by mass or more, more preferably 7.5 parts by mass or more, even more preferably 10 parts by

mass or more, most preferably 12 parts by mass or more, and is preferably 40 parts by mass or less, more preferably 30 parts by mass or less, even more preferably 20 parts by mass or less. If the content is less than 5 parts by mass, the effect of adding (d) the carboxylic acid and/or the salt thereof is not sufficient, and thus the linearity of the core hardness distribution may be lowered. If the content is more than 40 parts by mass, the resilience of the core may be lowered, since the hardness of the resultant core may be lowered as a whole.

In the case of using only the salt of the carboxylic acid as (d) the carboxylic acid and/or the salt thereof, it is more preferred that the content of the carboxylic acid is as follows. The content of (d) the salt of the carboxylic acid is preferably 10 parts by mass or more, more preferably 12 parts by mass or more, and is preferably less than 40 parts by mass, more preferably 30 parts by mass or less, even more preferably 25 parts by mass or less with respect to 100 parts by mass of (a) the base rubber. If the content is less than 10 parts by mass, the effect of adding (d) the salt of the carboxylic acid is not sufficient, and thus the linearity of the core hardness distribution may be lowered. If the content is 40 parts by mass or more, the resilience of the core may be lowered, since the hardness of the resultant core may be lowered as a whole.

There are cases where the surface of zinc acrylate used as the co-crosslinking agent is treated with stearic acid or zinc stearate to improve the dispersibility to the rubber. In the case of using zinc acrylate whose surface is treated with stearic acid or zinc stearate, in the present invention, the amount of stearic acid or zinc stearate used as a surface treating agent is included in the content of (d) the carboxylic acid and/or the salt thereof. For example, if 25 parts by mass of zinc acrylate whose surface treatment amount with stearic acid or zinc stearate is 10 mass % is used, the amount of stearic acid or zinc stearate is 2.5 parts by mass and the amount of zinc acrylate is 22.5 parts by mass. Thus, 2.5 parts by mass is counted as the content of (d) the carboxylic acid and/or the salt thereof.

Next, (e) the organic sulfur compound having a naphthalene ring will be explained. Use of (e) the organic sulfur compound having the naphthalene ring enhances a degree of the outer-hard and inner-soft structure while maintaining the linearity of the hardness distribution. There is no particular limitation on (e) the organic sulfur compound having the naphthalene ring, as long as it is an organic compound that has a naphthalene ring and a sulfur atom in a molecule thereof. Specific examples of (e) the organic sulfur compound having the naphthalene ring include, for example, thiophenols, thionaphthols, polysulfides, thiocarboxylic acids, dithiocarboxylic acids, sulfenamides, thiurams, dithiocarbamates, thiazoles, or salts thereof.

Examples of the metal salts are salts of monovalent metals such as sodium, lithium, potassium, copper (I), and silver (I), and salts of divalent metals such as zinc, magnesium, calcium, strontium, barium, titanium (II), manganese (II), iron (II), cobalt (II), nickel(II), zirconium(II), and tin (II).

As (e) the organic sulfur compound having the naphthalene ring, thionaphthol or derivatives thereof (hereinafter, collectively may be referred to as "thionaphthols") are preferable. The derivative of thionaphthol includes a metal salt thereof. Examples of thionaphthol or the derivative thereof are 2-naphthalenethiol, 1-naphthalenethiol, 2-chloro-1-naphthalenethiol, 2-bromo-1-naphthalenethiol, 2-fluoro-1-naphthalenethiol, 2-cyano-1-naphthalenethiol, 2-acetyl-1-naphthalenethiol, 1-chloro-2-naphthalenethiol, 1-bromo-2-naphthalenethiol, 1-fluoro-2-naphthalenethiol, 1-cyano-2-naphthalenethiol, and 1-acetyl-2-naphthalenethiol and metal

salts thereof. Preferable examples include 1-naphthalenethiol, 2-naphthalenethiol and zinc salt thereof.

The organic sulfur compounds may be used solely or as a mixture of at least two of them.

- 5 The content of (e) the organic sulfur compound having the naphthalene ring is preferably 0.05 part by mass or more, more preferably 0.1 part by mass or more, and is preferably 5.0 parts by mass or less, more preferably 2.0 parts by mass or less, with respect to 100 parts by mass of (a) the base rubber.
- 10 If the content of (e) the organic sulfur compound having the naphthalene ring is less than 0.05 part by mass, the effect of adding (e) the organic sulfur compound having the naphthalene ring cannot be obtained and thus the resilience may not improve. If the content of (e) the organic sulfur compound having the naphthalene ring exceeds 5.0 parts by mass, the compression deformation amount of the obtained golf ball becomes large and thus the resilience may be lowered.

- 15 In case of using the thionaphthols as (e) the organic sulfur compound having the naphthalene ring, the content of the thionaphthols is preferably 0.05 part by mass or more, more preferably 0.1 part by mass or more, and is preferably 2.0 parts by mass or less, more preferably 1.5 parts by mass or less with respect to 100 parts by mass of (a) the base rubber. If the content of the thionaphthols is less than 0.05 part by mass, the effect of adding the thionaphthols is not sufficient, and thus the resilience may not be improved. If the content exceeds 2.0 parts by mass, the compression deformation amount of the obtained golf ball becomes large and thus the resilience may be lowered.

- 20 The rubber composition used in the present invention may further include additives such as a pigment, a filler for adjusting weight or the like, an antioxidant, a peptizing agent, and a softener. Further, as described above, if the rubber composition used in the present invention contains only the  $\alpha,\beta$ -unsaturated carboxylic acid having 3 to 8 carbon atoms as a co-crosslinking agent, the rubber composition preferably contains (f) the metal compound.

- 25 (f) The metal compound is not limited as long as it can neutralize (b) the  $\alpha,\beta$ -unsaturated carboxylic acid having 3 to 8 carbon atoms in the rubber composition. Examples of (f) the metal compound include: metal hydroxides such as magnesium hydroxide, zinc hydroxide, calcium hydroxide, sodium hydroxide, lithium hydroxide, potassium hydroxide, copper hydroxide, or the like; metal oxides such as magnesium oxide, calcium oxide, zinc oxide, copper oxide, or the like; metal carbonates such as magnesium carbonate, zinc carbonate, calcium carbonate, sodium carbonate, lithium carbonate, potassium carbonate, or the like. Among them, (f) the metal compound preferably includes a bivalent metal compound, and more preferably includes a zinc compound. The bivalent metal compound reacts with the  $\alpha,\beta$ -unsaturated carboxylic acid having 3 to 8 carbon atoms, thereby forming a metal crosslinking. Further, use of the zinc compound provides a golf ball with excellent resilience. These (f) metal compounds may be used solely or as a mixture of at least two of them.

- 30 Examples of the pigment blended in the rubber composition include a white pigment, a blue pigment, and a purple pigment. As the white pigment, titanium oxide is preferably used. The type of titanium oxide is not particularly limited, but rutile type is preferably used because of the high opacity. The blending amount of titanium oxide is preferably 0.5 part by mass or more, and more preferably 2 parts by mass or more, and is preferably 8 parts by mass or less, and more preferably 5 parts by mass or less, with respect to 100 parts by mass of (a) the base rubber.

- 35 It is also preferred that the rubber composition contains both a white pigment and a blue pigment. The blue pigment is

## 11

blended in order to cause white color to be vivid, and examples thereof include ultramarine blue, cobalt blue, and phthalocyanine blue. Examples of the purple pigment include anthraquinone violet, dioxazine violet, and methyl violet.

The blending amount of the blue pigment is preferably 0.001 part by mass or more, and more preferably 0.05 part by mass or more, and is preferably 0.2 part by mass or less, and more preferably 0.1 part by mass or less, with respect to 100 parts by mass of (a) the base rubber. If the blending amount of the blue pigment is less than 0.001 part by mass, blueness is insufficient, and the color looks yellowish. If the blending amount of the blue pigment exceeds 0.2 part by mass, blueness is excessively strong, and a vivid white appearance is not provided.

The filler blended in the rubber composition is used as a weight adjusting agent for mainly adjusting the weight of the golf ball obtained as a final product. The filler may be blended where necessary. The filler includes, for example, inorganic fillers such as zinc oxide, barium sulfate, calcium carbonate, magnesium oxide, tungsten powder, molybdenum powder, or the like. The content of the filler is preferably 0.5 part by mass or more, more preferably 1 part by mass or more, and is preferably 30 parts by mass or less, more preferably 25 parts by mass or less, even more preferably 20 parts by mass or less. If the content of the filler is less than 0.5 part by mass, it is difficult to adjust the weight, while if the content of the filler exceeds 30 parts by mass, the weight ratio of the rubber component becomes small and thus the resilience tends to be lowered.

The blending amount of the antioxidant is preferably 0.1 part by mass or more and 1 part by mass or less, with respect to 100 parts by mass of (a) the base rubber. In addition, the blending amount of the peptizing agent is preferably 0.1 part by mass or more and 5 parts by mass or less, with respect to 100 parts by mass of (a) the base rubber.

The rubber composition used in the present invention is obtained by mixing and kneading (a) the base rubber, (b) the  $\alpha, \beta$ -unsaturated carboxylic acid having 3 to 8 carbon atoms and/or the metal salt thereof, (c) the crosslinking initiator, and (d) the carboxylic acid and/or the salt thereof, and (e) organic sulfur compound having the naphthalene ring. The kneading can be conducted, without any limitation, with a well-known kneading machine such as a kneading roll, a banbury mixer, a kneader, or the like.

The spherical core of the golf ball of the present invention can be obtained by molding the rubber composition after kneaded. The spherical core of the golf ball of the present invention can be obtained by molding the kneaded rubber composition in the mold. For example, the press-molding is preferably carried out for 10 to 60 minutes at the temperature of 130° C. to 200° C. under the pressure of 2.9 MPa to 11.8 MPa. Alternatively, the press-molding is preferably carried out in a two-step heating, for example, for 20 to 40 minutes at the temperature of 130° C. to 150° C., and continuously for 5 to 15 minutes at the temperature of 160° C. to 180° C. In the present invention, it is preferred to select the molding conditions where the spherical core has a desired hardness distribution. In the present invention, it is preferable to select the molding condition in order to make the spherical core have a desired hardness distribution.

In a preferable embodiment, when the hardness is measured at nine points obtained by dividing a radius of the spherical core into equal parts having 12.5% interval and the hardness is plotted against distance (%) from the center of the spherical core, the spherical core is such that  $R^2$  of a linear approximation curve obtained by the least square method is 0.95 or higher. That is, JIS-C hardness is measured at nine

## 12

points, namely at distances of 0% (core center), 12.5%, 25%, 37.5%, 50%, 62.5%, 75%, 87.5%, 100% (core surface) from the core center. Next, the measurement results are plotted to make a graph having JIS-C hardness as a vertical axis and 5 distances (%) from the core center as a horizontal axis. In the present invention,  $R^2$  of a linear approximation curve obtained from this graph by the least square method is 0.95 or higher.  $R^2$  of the linear approximation curve obtained by the least square method indicates the linearity of the obtained 10 plot.  $R^2$  of 0.95 or more means that the core has the hardness distribution where the hardness increases linearly or almost linearly. In the present invention, since the hardness of the spherical core is JIS-C hardness measured at nine points obtained by dividing a radius of the spherical core into equal 15 parts having 12.5% interval, the accuracy of the linearity of the core hardness distribution becomes extremely high. If the core having the hardness distribution where the hardness increases linearly or almost linearly is used for the golf ball, the spin rate on driver shots decrease. As a result, the flight 20 distance on driver shots increases.  $R^2$  of the linear approximation curve is preferably 0.96 or more. The higher linearity provides a greater flight distance on driver shots.

The spherical core preferably has a hardness difference (Hs-H0) between a surface hardness Hs and a center hardness 25 H0 of 15 or more, more preferably 18 or more, even more preferably 22 or more, and preferably has a hardness difference of 50 or less, more preferably 45 or less, even more preferably 40 or less in JIS-C hardness. If the hardness difference between the center hardness and the surface hardness 30 is large, the golf ball traveling a great flight distance due to the high launch angle and low spin rate is obtained.

The spherical core preferably has the center hardness H0 of 30 or more, more preferably 40 or more, even more preferably 45 or more, most preferably 50 or more in JIS-C hardness. If the center hardness H0 is less than 30 in JIS-C hardness, the core becomes too soft and thus the resilience may be lowered. Further, the spherical core has the center hardness H0 of 70 or less, more preferably 65 or less. If the center hardness H0 exceeds 70 in JIS-C hardness, the core becomes too hard and 40 thus the shot feeling tends to be lowered.

The spherical core preferably has the surface hardness Hs of 78 or more, more preferably 80 or more, and has preferably has the surface hardness Hs of 100 or less, more preferably 95 or less, even more preferably 90 or less in JIS-C hardness. If the surface hardness is 78 or more in JIS-C hardness, the spherical core does not become excessively soft, and thus the better resilience is obtained. Further, if the surface hardness of the spherical core is 100 or less in JIS-C hardness, the spherical core does not become excessively hard, and thus the better shot feeling is obtained.

The spherical core preferably has the diameter of the 34.8 mm or more, more preferably 36.8 mm or more, and even more preferably 38.8 mm or more, and preferably has the diameter of 42.2 mm or less, more preferably 41.8 mm or less, 55 and even more preferably 41.2 mm or less, and most preferably 40.8 mm or less. If the spherical core has the diameter of 34.8 mm or more, the thickness of the cover does not become too thick and thus the resilience becomes better. On the other hand, if the spherical core has the diameter of 42.2 mm or less, the thickness of the cover does not become too thin, and hence the cover functions better.

When the spherical core has a diameter from 34.8 mm to 42.2 mm, a compression deformation amount (shrinking deformation amount of the spherical core along the compression direction) of the spherical core when applying a load from 98 N as an initial load to 1275 N as a final load is 60 preferably 2.0 mm or more, more preferably 2.8 mm or more,

and is preferably 6.0 mm or less, more preferably 4.5 mm or less. If the compression deformation amount is 2.0 mm or more, the shot feeling of the golf ball becomes better. If the compression deformation amount is 6.0 mm or less, the resilience of the golf ball becomes better.

The golf ball cover of the present invention is formed from a cover composition comprising a resin component. Examples of the resin component include, for example, an ionomer rein; a thermoplastic polyurethane elastomer having a commercial name of "Elastollan (e.g. "Elastollan XNY85A")" commercially available from BASF Japan Ltd; a thermoplastic polyamide elastomer having a commercial name of "Pebax (e.g. "Pebax 2533")" commercially available from Arkema K. K.; a thermoplastic polyester elastomer having a commercial name of "Hytrel (e.g. "Hytrel 3548", "Hytrel 4047")" commercially available from Du Pont-Toray Co., Ltd.; and a thermoplastic styrene elastomer having a commercial name of "Rabalon (e.g. "Rabalon T3221C")" commercially available from Mitsubishi Chemical Corporation; and the like.

The ionomer resin includes a product prepared by neutralizing at least a part of carboxyl groups in the binary copolymer composed of an olefin and an  $\alpha,\beta$ -unsaturated carboxylic acid having 3 to 8 carbon atoms with a metal ion, a product prepared by neutralizing at least a part of carboxyl groups in the ternary copolymer composed of an olefin, an  $\alpha,\beta$ -unsaturated carboxylic acid having 3 to 8 carbon atoms, and an  $\alpha,\beta$ -unsaturated carboxylic acid ester with a metal ion, or a mixture of those. The olefin preferably includes an olefin having 2 to 8 carbon atoms. Examples of the olefin are ethylene, propylene, butene, pentene, hexene, heptene, and octene. The olefin more preferably includes ethylene. Examples of the  $\alpha,\beta$ -unsaturated carboxylic acid having 3 to 8 carbon atoms are acrylic acid, methacrylic acid, fumaric acid, maleic acid and crotonic acid. Among these, acrylic acid and methacrylic acid are particularly preferred. Examples of the  $\alpha,\beta$ -unsaturated carboxylic acid ester include methyl ester, ethyl ester, propyl ester, n-butyl ester, isobutyl ester of acrylic acid, methacrylic acid, fumaric acid, maleic acid or the like. In particular, acrylic acid ester and methacrylic acid ester are preferable. Among these, the ionomer resin preferably includes the metal ion-neutralized product of the binary copolymer composed of ethylene-(meth)acrylic acid and the metal ion-neutralized product of the ternary copolymer composed of ethylene, (meth)acrylic acid, and (meth)acrylic acid ester.

Specific examples of the ionomer resins include trade name "Himilan (registered trademark) (e.g. the binary copolymerized ionomer such as Himilan 1555 (Na), Himilan 1557 (Zn), Himilan 1605 (Na), Himilan 1706 (Zn), Himilan 1707 (Na), Himilan AM7311 (Mg), Himilan AM7329 (Zn); and the ternary copolymerized ionomer such as Himilan 1856 (Na), Himilan 1855 (Zn))" commercially available from Du Pont-Mitsui Polymers Co., Ltd.

Further, examples include "Surlyn (registered trademark) (e.g. the binary copolymerized ionomer such as Surlyn 8945 (Na), Surlyn 9945 (Zn), Surlyn 8140 (Na), Surlyn 8150 (Na), Surlyn 9120 (Zn), Surlyn 9150 (Zn), Surlyn 6910 (Mg), Surlyn 6120 (Mg), Surlyn 7930 (Li), Surlyn 7940 (Li), Surlyn AD8546 (Li); and the ternary copolymerized ionomer such as Surlyn 6320 (Mg), Surlyn 8120 (Na), Surlyn 8320 (Na), Surlyn 9320 (Zn), HPF 1000 (Mg), HPF 2000 (Mg))" commercially available from E.I. du Pont de Nemours and Company.

Further, examples include "Iotek (registered trademark) (e.g. the binary copolymerized ionomer such as Iotek 8000 (Na), Iotek 8030 (Na), Iotek 7010 (Zn), Iotek 7030 (Zn); and

the ternary copolymerized ionomer such as Iotek 7510 (Zn), Iotek 7520 (Zn))" commercially available from ExxonMobil Chemical Corporation.

It is noted that Na, Zn, Li, and Mg described in the parentheses after the trade names indicate metal types of neutralizing metal ions for the ionomer resins.

The cover composition constituting the cover of the golf ball of the present invention preferably includes, as a resin component, a thermoplastic polyurethane elastomer or an ionomer rein. In case of using the ionomer rein, it is preferred to use a thermoplastic styrene elastomer together. The content of the polyurethane or ionomer resin in resin component of the cover composition is preferably 50 mass % or more, more preferably 60 mass % or more, even more preferably 70 mass % or more.

In the present invention, the cover composition may further contain a pigment component such as a white pigment (for example, titanium oxide), a blue pigment, and a red pigment; a weight adjusting agent such as zinc oxide, calcium carbonate, and barium sulfate; a dispersant; an antioxidant; an ultraviolet absorber; a light stabilizer; a fluorescent material or a fluorescent brightener; and the like, as long as they do not impair the effect of the present invention.

The amount of the white pigment (for example, titanium oxide) is preferably 0.5 part or more, more preferably 1 part or more, and the content of the white pigment is preferably 10 parts or less, more preferably 8 parts or less, with respect to 100 parts of the resin component constituting the cover by mass. If the amount of the white pigment is 0.5 part by mass or more, it is possible to impart the opacity to the resultant cover. Further, if the amount of the white pigment is more than 10 parts by mass, the durability of the resultant cover may deteriorate.

The slab hardness of the cover composition is preferably set in accordance with the desired performance of the golf balls. For example, in case of a so-called distance golf ball which focuses on a flight distance, the cover composition preferably has a slab hardness of 50 or more, more preferably 55 or more, and preferably has a slab hardness of 80 or less, more preferably 70 or less in shore D hardness. If the cover composition has a slab hardness of 50 or more, the obtained golf ball has a high launch angle and low spin rate on driver shots and iron shots, and thus the flight distance improves. If the cover composition has a slab hardness of 80 or less, the golf ball excellent in durability is obtained. Further, in case of a so-called spin golf ball which focuses on controllability, the cover composition preferably has a slab hardness of less than 50, and preferably has a slab hardness of 20 or more, more preferably 25 or more in shore D hardness. If the cover composition has a slab hardness of less than 50, the flight distance on driver shots can be improved by the core of the present invention, as well as the obtained golf ball readily stops on the green due to the high spin rate on approach shots. If the cover composition has a slab hardness of 20 or more, the abrasion resistance improves. In case of a plurality of cover layers, the slab hardness of the cover composition constituting each layer can be identical or different, as long as the slab hardness of each layer is within the above range.

An embodiment for molding a cover is not particularly limited, and includes an embodiment which comprises injection molding the cover composition directly onto the core, or an embodiment which comprises molding the cover composition into a hollow-shell, covering the core with a plurality of the hollow-shells and subjecting the core with a plurality of the hollow shells to the compression-molding (preferably an embodiment which comprises molding the cover composition into a half hollow-shell, covering the core with the two

half hollow-shells, and subjecting the core with the two half hollow-shells to the compression-molding).

When molding the cover in a compression molding method, molding of the half shell can be performed by either compression molding method or injection molding method, and the compression molding method is preferred. The compression-molding of the cover composition into half shell can be carried out, for example, under a pressure of 1 MPa or more and 20 MPa or less at a temperature of  $-20^{\circ}\text{C}$ . or more and  $70^{\circ}\text{C}$ . or less relative to the flow beginning temperature of the cover composition. By performing the molding under the above conditions, a half shell having a uniform thickness can be formed. Examples of a method for molding the cover using half shells include compression molding by covering the core with two half shells. The compression molding of half shells into the cover can be carried out, for example, under a pressure of 0.5 MPa or more and 25 MPa or less at a temperature of  $-20^{\circ}\text{C}$ . or more and  $70^{\circ}\text{C}$ . or less relative to the flow beginning temperature of the cover composition. By performing the molding under the above conditions, a golf ball cover having a uniform thickness can be formed.

In the case of directly injection molding the cover composition, the cover composition extruded in the pellet form beforehand may be used for injection molding or the materials such as the base resin components and the pigment may be dry blended, followed by directly injection molding the blended material. It is preferred to use upper and lower molds having a spherical cavity and pimples for forming a cover, wherein a part of the pimples also serves as a retractable hold pin. When molding the cover by injection molding, the hold pin is protruded to hold the core, and the cover composition which has been heated and melted is charged and then cooled to obtain a cover. For example, it is preferred that the cover composition heated and melted at the temperature ranging from  $200^{\circ}\text{C}$ . to  $250^{\circ}\text{C}$ . is charged into a mold held under the pressure of 9 MPa to 15 MPa for 0.5 to 5 seconds, and after cooling for 10 to 60 seconds, the mold is opened and the golf ball with the cover molded is taken out from the mold.

The concave portions called "dimple" are usually formed on the surface of the cover, when molding the cover. The total number of the dimples formed on the cover is preferably 200 or more and 500 or less. If the total number is less than 200, the dimple effect is hardly obtained. On the other hand, if the total number exceeds 500, the dimple effect is hardly obtained because the size of the respective dimples is small. The shape (shape in a plan view) of dimples includes, for example, without limitation, a circle, polygonal shapes such as roughly triangular shape, roughly quadrangular shape, roughly pentagonal shape, roughly hexagonal shape, and another irregular shape. The shape of the dimples is employed solely or at least two of them may be used in combination.

In the present invention, the thickness of the cover of the golf ball is preferably 4.0 mm or less, more preferably 3.0 mm or less, even more preferably 2.0 mm or less. If the thickness of the cover is 4.0 mm or less, the resilience and shot feeling of the obtained golf ball become better. The thickness of the cover is preferably 0.3 mm or more, more preferably 0.5 mm or more, and even more preferably 0.8 mm or more, and most preferably 1.0 mm or more. If the thickness of the cover is less than 0.3 mm, the durability and the wear resistance of the cover may deteriorate. If the cover has a plurality of layers, it is preferred that the total thickness of the cover layers falls within the above range.

After the cover is molded, the mold is opened and the golf ball body is taken out from the mold, and as necessary, the golf ball body is preferably subjected to surface treatments such as deburring, cleaning, and sandblast. If desired, a paint

film or a mark may be formed. The paint film preferably has a thickness of, but not limited to, 5  $\mu\text{m}$  or larger, and more preferably 7  $\mu\text{m}$  or larger, and preferably has a thickness of 50  $\mu\text{m}$  or smaller, and more preferably 40  $\mu\text{m}$  or smaller, even more preferably 30  $\mu\text{m}$  or smaller. If the thickness is smaller than 5  $\mu\text{m}$ , the paint film is easy to wear off due to continued use of the golf ball, and if the thickness is larger than 50  $\mu\text{m}$ , the effect of the dimples is reduced, resulting in lowering flying performance of the golf ball.

When the golf ball of the present invention has a diameter in a range from 40 mm to 45 mm, a compression deformation amount of the golf ball (shrinking amount of the golf ball in the compression direction thereof) when applying a load from an initial load of 98 N to a final load of 1275 N to the golf ball is preferably 2.0 mm or more, more preferably 2.4 mm or more, even more preferably 2.5 mm or more, most preferably 2.8 mm or more, and is preferably 4.0 mm or less, more preferably 3.8 mm or less, even more preferably 3.6 mm or less. If the compression deformation amount is 2.0 mm or more, the golf ball does not become excessively hard, and thus exhibits the good shot feeling. On the other hand, if the compression deformation amount is 4.0 mm or less, the resilience is enhanced.

The golf ball construction is not limited, as long as the golf ball of the present invention comprises a spherical core and at least one cover layer covering the spherical core. The spherical core preferably has a single layered structure. Unlike the multi-layered structure, the spherical core of the single layered structure does not have an energy loss at the interface of the multi-layered structure when hitting, and thus has an improved resilience. The cover has a structure of at least one layer, for example a single layered structure, or a multi-layered structure of at least two layers. The golf ball of the present invention includes, for example, a two-piece golf ball comprising a spherical core and a single layered cover disposed around the spherical core, a multi-piece golf ball comprising a spherical core, and at least two cover layers disposed around the spherical core (including the three-piece golfball), and a wound golf ball comprising a spherical core, a rubber thread layer which is formed around the spherical core, and a cover disposed over the rubber thread layer. The present invention can be suitably applied to any one of the above golf balls.

## EXAMPLES

Hereinafter, the present invention will be described in detail by way of example. The present invention is not limited to examples described below. Various changes and modifications can be made without departing from the spirit and scope of the present invention.

### [Evaluation Methods]

#### (1) Compression Deformation Amount (mm)

A compression deformation amount of the core or golf ball (a shrinking amount of the core or golf ball in the compression direction thereof), when applying a load from 98 N as an initial load to 1275 N as a final load to the core or golf ball, was measured.

#### (2) Coefficient of Restitution

A 198.4 g of metal cylindrical object was allowed to collide with each core or golf ball at a speed of 40 m/sec, and the speeds of the cylindrical object and the core or golf ball before and after the collision were measured. Based on these speeds and the mass of each object, coefficient of restitution for each core or golf ball was calculated. The measurement was conducted by using twelve samples for each core or golf ball, and the average value was regarded as the coefficient of restitution

for the core or golf ball. The coefficient of restitution of golf balls No. 1 to No. 13 are shown as the difference from that of the golf ball No. 13. The coefficient of restitution of golf balls No. 14 to 26 are shown as the difference from that of the golf ball No. 16.

(3) Slab Hardness (Shore D Hardness)

Sheets with a thickness of about 2 mm were produced by injection molding the cover composition, and stored at 23° C. for two weeks. Three or more of these sheets were stacked on one another so as not to be affected by the measuring substrate on which the sheets were placed, and the hardness of the stack was measured with a type P1 auto loading durometer manufactured by Kobunshi Keiki Co., Ltd., provided with a Shore D type spring hardness tester prescribed in ASTM-D2240.

(4) Hardness Distribution of Spherical Core (JIS-C Hardness)

A type P1 auto loading durometer manufactured by Kobunshi Keiki Co., Ltd., provided with a JIS-C type spring hardness tester was used to measure the hardness of the spherical core. The hardness measured at the surface of the spherical core was adopted as the surface hardness of the spherical core. The spherical core was cut into two hemispheres to obtain a cut plane, and the hardness were measured at the central point and at predetermined distances from the central point. The core hardness were measured at 4 points at predetermined distances from the central point of the cut

plane of the core. JIS-C hardness was calculated by averaging the hardness measured at 4 points at predetermined distances from the center of the core.

(5) Flight Distance (m) and Spin Rate (rpm) on a Driver Shot

A metal-headed W#1 driver (XXIO S, loft: 11°, manufactured by SRI Sports Limited) was installed on a swing robot M/C manufactured by Golf Laboratories, Inc. A golf ball was hit at a head speed of 40 m/sec, and the flight distance (the distance from the launch point to the stop point) and the spin rate immediately after hitting the golf ball were measured.

This measurement was conducted twelve times for each golf ball, and the average value was adopted as the measurement value for the golf ball. A sequence of photographs of the hit golf ball was taken for measuring the spin rate (rpm) immediately after hitting the golf ball. The flight distance and spin rate on the driver shots of golf balls No. 1 to No. 13 are shown as the difference from those of the golf ball No. 13. The flight distance and spin rate on the driver shots of golf balls No. 14 to 26 are shown as the difference from those of the golf ball No. 16.

[Production of Cores]

The rubber compositions having formulations shown in Tables 3 to 6 were kneaded and heat-pressed in upper and lower molds, each having a hemispherical cavity, at 170° C. for 20 minutes to prepare spherical cores having a diameter of 39.8 mm. The hardness distributions of the obtained spherical core No. 1 to No. 26 are shown in FIGS. 1 to 12.

TABLE 3

|                                          |                                      | Golf ball No. |       |       |       |       |       |
|------------------------------------------|--------------------------------------|---------------|-------|-------|-------|-------|-------|
|                                          |                                      | 1             | 2     | 3     | 4     | 5     | 6     |
| Rubber composition                       | BR730                                | 100           | 100   | 100   | 100   | 100   | 100   |
| (parts by mass)                          | Sanceler SR                          | 28            | 28    | 24    | 30    | 24    | 28    |
|                                          | Zinc oxide                           | 5             | 5     | 5     | 5     | 5     | 5     |
|                                          | Barium sulfate                       | *1)           | *1)   | *1)   | *1)   | *1)   | *1)   |
|                                          | 2-Thionaphthol                       | 0.32          | 0.32  | 0.1   | 0.5   | 0.1   | 0.32  |
|                                          | Stearic acid                         | 10            | 10    | 10    | 10    | —     | —     |
|                                          | Zinc stearate                        | —             | —     | —     | —     | 10    | 10    |
|                                          | Myristic acid                        | —             | —     | —     | —     | —     | —     |
|                                          | Dicumyl peroxide                     | 0.8           | 0.8   | 0.8   | 0.8   | 0.8   | 0.8   |
|                                          | Total amount of carboxylic acid/salt | 12.8          | 12.8  | 12.4  | 13.0  | 12.4  | 12.8  |
| Core hardness distribution (JIS-C)       | Center hardness                      | 54.2          | 54.2  | 52.1  | 53.2  | 47.9  | 54.4  |
|                                          | 12.5% point hardness                 | 58.2          | 58.2  | 60.6  | 58.5  | 55.4  | 60.2  |
|                                          | 25% point hardness                   | 62.5          | 62.5  | 64.7  | 62.3  | 61.6  | 64.4  |
|                                          | 37.5% point hardness                 | 65.1          | 65.1  | 67.9  | 64.8  | 65.1  | 67.2  |
|                                          | 50% point hardness                   | 65.9          | 65.9  | 69.7  | 65.2  | 66.8  | 68.3  |
|                                          | 62.5% point hardness                 | 70.0          | 70.0  | 70.1  | 68.3  | 69.3  | 70.5  |
|                                          | 75% point hardness                   | 77.7          | 77.7  | 75.1  | 75.3  | 75.4  | 77.6  |
|                                          | 87.5% point hardness                 | 80.7          | 80.7  | 77.9  | 78.3  | 79.1  | 80.6  |
|                                          | Surface hardness                     | 83.6          | 83.6  | 83.4  | 83.2  | 84.3  | 83.9  |
|                                          | Surface hardness – center hardness   | 29.4          | 29.4  | 31.3  | 30.0  | 36.4  | 29.5  |
|                                          | R <sup>2</sup> of approximated curve | 0.98          | 0.98  | 0.95  | 0.97  | 0.98  | 0.98  |
|                                          | Slope of approximated curve          | 0.29          | 0.29  | 0.27  | 0.28  | 0.33  | 0.28  |
| Core coefficient of restitution          |                                      | 0.016         | 0.016 | 0.010 | 0.009 | 0.006 | 0.007 |
| Core compression deformation amount (mm) |                                      | 3.94          | 3.94  | 3.91  | 4.16  | 4.09  | 3.83  |
| Cover composition                        |                                      | A             | B     | A     | A     | A     | A     |
| Cover hardness (Shore D)                 |                                      | 65            | 55    | 65    | 65    | 65    | 65    |
| Cover thickness (mm)                     |                                      | 1.5           | 1.5   | 1.5   | 1.5   | 1.5   | 1.5   |
| Ball                                     | Driver spin rate (rpm)               | -90           | -20   | -40   | -70   | -120  | -80   |
|                                          | Driver flying distance (m)           | 3.8           | 2.6   | 2.1   | 2.4   | 4.0   | 2.9   |
|                                          | Coefficient of restitution           | 0.016         | 0.011 | 0.010 | 0.009 | 0.006 | 0.007 |
|                                          | Compression deformation amount (mm)  | 3.24          | 3.34  | 3.21  | 3.46  | 3.39  | 3.13  |

TABLE 4

|                                          |                                                                                                                                                                                                                                                                                                           | Golf ball No.                                                                                |                                                                                              |                                                                                              |                                                                                              |                                                                                              |                                                                                              |                                                                                              |
|------------------------------------------|-----------------------------------------------------------------------------------------------------------------------------------------------------------------------------------------------------------------------------------------------------------------------------------------------------------|----------------------------------------------------------------------------------------------|----------------------------------------------------------------------------------------------|----------------------------------------------------------------------------------------------|----------------------------------------------------------------------------------------------|----------------------------------------------------------------------------------------------|----------------------------------------------------------------------------------------------|----------------------------------------------------------------------------------------------|
|                                          |                                                                                                                                                                                                                                                                                                           | 7                                                                                            | 8                                                                                            | 9                                                                                            | 10                                                                                           | 11                                                                                           | 12                                                                                           | 13                                                                                           |
| Rubber composition (parts by mass)       | BR730<br>Sanceler SR                                                                                                                                                                                                                                                                                      | 100<br>28                                                                                    | 100<br>30                                                                                    | 100<br>5                                                                                     | 100<br>5                                                                                     | 100<br>5                                                                                     | 100<br>5                                                                                     | 100<br>5                                                                                     |
| Zinc oxide                               |                                                                                                                                                                                                                                                                                                           | 5                                                                                            | 5                                                                                            | 5                                                                                            | 5                                                                                            | 5                                                                                            | 5                                                                                            | 5                                                                                            |
| Barium sulfate                           |                                                                                                                                                                                                                                                                                                           | *1)<br>0.5                                                                                   | *1)<br>0.32                                                                                  | *1)<br>0.32                                                                                  | *1)<br>0.1                                                                                   | *1)<br>0.5                                                                                   | *1)<br>2                                                                                     | *1)<br>—                                                                                     |
| 2-Thionaphthol                           |                                                                                                                                                                                                                                                                                                           |                                                                                              |                                                                                              |                                                                                              |                                                                                              |                                                                                              |                                                                                              |                                                                                              |
| Stearic acid                             |                                                                                                                                                                                                                                                                                                           | —                                                                                            | —                                                                                            | —                                                                                            | —                                                                                            | —                                                                                            | —                                                                                            | —                                                                                            |
| Zinc stearate                            |                                                                                                                                                                                                                                                                                                           | 10                                                                                           | —                                                                                            | —                                                                                            | —                                                                                            | —                                                                                            | —                                                                                            | —                                                                                            |
| Myristic acid                            |                                                                                                                                                                                                                                                                                                           | —                                                                                            | 10                                                                                           | —                                                                                            | —                                                                                            | —                                                                                            | —                                                                                            | —                                                                                            |
| Dicumyl peroxide                         |                                                                                                                                                                                                                                                                                                           | 0.8                                                                                          | 0.8                                                                                          | 0.8                                                                                          | 0.8                                                                                          | 0.8                                                                                          | 0.8                                                                                          | 0.8                                                                                          |
| Total amount of carboxylic acid/salt     |                                                                                                                                                                                                                                                                                                           | 12.8                                                                                         | 13.0                                                                                         | 3.0                                                                                          | 2.4                                                                                          | 3.0                                                                                          | 3.8                                                                                          | 2.3                                                                                          |
| Core hardness distribution (JIS-C)       | Center hardness<br>12.5% point hardness<br>25% point hardness<br>37.5% point hardness<br>50% point hardness<br>62.5% point hardness<br>75% point hardness<br>87.5% point hardness<br>Surface hardness<br>Surface hardness – center hardness<br>$R^2$ of approximated curve<br>Slope of approximated curve | 49.4<br>54.2<br>58.2<br>60.6<br>62.0<br>66.6<br>73.6<br>75.9<br>80.7<br>31.3<br>0.98<br>0.30 | 49.6<br>53.0<br>56.5<br>58.9<br>60.0<br>66.1<br>74.5<br>77.1<br>81.0<br>31.4<br>0.97<br>0.32 | 56.5<br>62.0<br>65.9<br>67.0<br>66.8<br>66.5<br>73.4<br>79.0<br>84.1<br>27.6<br>0.89<br>0.23 | 57.6<br>63.6<br>68.2<br>69.3<br>69.6<br>68.4<br>75.1<br>82.5<br>86.9<br>29.3<br>0.89<br>0.25 | 53.0<br>61.2<br>66.9<br>67.8<br>67.8<br>69.1<br>74.5<br>79.0<br>82.7<br>29.7<br>0.92<br>0.25 | 52.0<br>59.2<br>64.9<br>66.8<br>65.8<br>69.1<br>73.5<br>77.0<br>80.7<br>28.7<br>0.94<br>0.25 | 57.7<br>63.2<br>66.5<br>67.7<br>67.7<br>68.2<br>73.5<br>76.1<br>81.4<br>23.7<br>0.92<br>0.20 |
| Core coefficient of restitution          |                                                                                                                                                                                                                                                                                                           | 0.005                                                                                        | 0.012                                                                                        | 0.012                                                                                        | 0.007                                                                                        | 0.004                                                                                        | -0.001                                                                                       | 0.000                                                                                        |
| Core compression deformation amount (mm) |                                                                                                                                                                                                                                                                                                           | 4.39                                                                                         | 4.12                                                                                         | 4.06                                                                                         | 4.00                                                                                         | 4.17                                                                                         | 4.33                                                                                         | 4.29                                                                                         |
| Cover composition                        |                                                                                                                                                                                                                                                                                                           | A                                                                                            | A                                                                                            | A                                                                                            | A                                                                                            | A                                                                                            | A                                                                                            | A                                                                                            |
| Cover hardness (Shore D)                 |                                                                                                                                                                                                                                                                                                           | 65                                                                                           | 65                                                                                           | 65                                                                                           | 65                                                                                           | 65                                                                                           | 65                                                                                           | 65                                                                                           |
| Cover thickness (mm)                     |                                                                                                                                                                                                                                                                                                           | 1.5                                                                                          | 1.5                                                                                          | 1.5                                                                                          | 1.5                                                                                          | 1.5                                                                                          | 1.5                                                                                          | 1.5                                                                                          |
| Ball                                     | Driver spin rate (rpm)<br>Driver flying distance (m)<br>Coefficient of restitution<br>Compression deformation amount (mm)                                                                                                                                                                                 | -100<br>3.5<br>0.005<br>3.69                                                                 | -80<br>2.5<br>0.012<br>3.42                                                                  | -10<br>0.8<br>0.009<br>3.36                                                                  | -20<br>0<br>0.009<br>3.30                                                                    | -30<br>0.6<br>0.004<br>3.47                                                                  | -30<br>0.2<br>-0.001<br>3.63                                                                 | 0<br>0<br>0<br>3.59                                                                          |

TABLE 5

|                                          |                                                                                                                                                                                                                                                                                                           | Golf ball No.                                                                                |                                                                                              |                                                                                              |                                                                                              |                                                                                              |                                                                                              |
|------------------------------------------|-----------------------------------------------------------------------------------------------------------------------------------------------------------------------------------------------------------------------------------------------------------------------------------------------------------|----------------------------------------------------------------------------------------------|----------------------------------------------------------------------------------------------|----------------------------------------------------------------------------------------------|----------------------------------------------------------------------------------------------|----------------------------------------------------------------------------------------------|----------------------------------------------------------------------------------------------|
|                                          |                                                                                                                                                                                                                                                                                                           | 14                                                                                           | 15                                                                                           | 16                                                                                           | 17                                                                                           | 18                                                                                           | 19                                                                                           |
| Rubber composition (parts by mass)       | BR730<br>Sanceler SR                                                                                                                                                                                                                                                                                      | 100<br>28                                                                                    | 100<br>28                                                                                    | 100<br>24                                                                                    | 100<br>30                                                                                    | 100<br>24                                                                                    | 100<br>28                                                                                    |
| Zinc oxide                               |                                                                                                                                                                                                                                                                                                           | 5                                                                                            | 5                                                                                            | 5                                                                                            | 5                                                                                            | 5                                                                                            | 5                                                                                            |
| Barium sulfate                           |                                                                                                                                                                                                                                                                                                           | *1)<br>0.32                                                                                  | *1)<br>0.32                                                                                  | *1)<br>0.1                                                                                   | *1)<br>0.5                                                                                   | *1)<br>0.1                                                                                   | *1)<br>0.32                                                                                  |
| 2-Thionaphthol                           |                                                                                                                                                                                                                                                                                                           |                                                                                              |                                                                                              |                                                                                              |                                                                                              |                                                                                              |                                                                                              |
| Stearic acid                             |                                                                                                                                                                                                                                                                                                           | 10                                                                                           | 10                                                                                           | 10                                                                                           | 10                                                                                           | —                                                                                            | —                                                                                            |
| Zinc stearate                            |                                                                                                                                                                                                                                                                                                           | —                                                                                            | —                                                                                            | —                                                                                            | —                                                                                            | 10                                                                                           | 10                                                                                           |
| Myristic acid                            |                                                                                                                                                                                                                                                                                                           | —                                                                                            | —                                                                                            | —                                                                                            | —                                                                                            | —                                                                                            | —                                                                                            |
| Dicumyl peroxide                         |                                                                                                                                                                                                                                                                                                           | 0.8                                                                                          | 0.8                                                                                          | 0.8                                                                                          | 0.8                                                                                          | 0.8                                                                                          | 0.8                                                                                          |
| Total amount of carboxylic acid/salt     |                                                                                                                                                                                                                                                                                                           | 12.8                                                                                         | 12.8                                                                                         | 12.4                                                                                         | 13.0                                                                                         | 12.4                                                                                         | 12.8                                                                                         |
| Core hardness distribution (JIS-C)       | Center hardness<br>12.5% point hardness<br>25% point hardness<br>37.5% point hardness<br>50% point hardness<br>62.5% point hardness<br>75% point hardness<br>87.5% point hardness<br>Surface hardness<br>Surface hardness – center hardness<br>$R^2$ of approximated curve<br>Slope of approximated curve | 54.2<br>58.2<br>62.5<br>65.1<br>65.9<br>70.0<br>77.7<br>80.7<br>83.6<br>29.4<br>0.98<br>0.29 | 54.2<br>58.2<br>62.5<br>65.1<br>65.9<br>70.0<br>77.7<br>80.7<br>83.6<br>29.4<br>0.98<br>0.29 | 52.1<br>58.5<br>64.7<br>67.9<br>69.7<br>70.1<br>75.1<br>77.9<br>83.4<br>31.3<br>0.95<br>0.27 | 53.2<br>58.5<br>62.3<br>64.8<br>65.2<br>68.3<br>75.3<br>78.3<br>83.2<br>30.0<br>0.97<br>0.28 | 47.9<br>55.4<br>61.6<br>65.1<br>66.8<br>69.3<br>75.4<br>79.1<br>84.3<br>36.4<br>0.98<br>0.33 | 54.4<br>60.2<br>64.4<br>67.2<br>68.3<br>70.5<br>77.6<br>80.6<br>83.9<br>29.5<br>0.98<br>0.28 |
| Core coefficient of restitution          |                                                                                                                                                                                                                                                                                                           | 0.016                                                                                        | 0.016                                                                                        | 0.010                                                                                        | 0.009                                                                                        | 0.006                                                                                        | 0.007                                                                                        |
| Core compression deformation amount (mm) |                                                                                                                                                                                                                                                                                                           | 3.94                                                                                         | 3.94                                                                                         | 3.91                                                                                         | 4.16                                                                                         | 4.09                                                                                         | 3.83                                                                                         |
| Cover composition                        |                                                                                                                                                                                                                                                                                                           | C                                                                                            | D                                                                                            | C                                                                                            | C                                                                                            | C                                                                                            | C                                                                                            |
| Cover hardness (Shore D)                 |                                                                                                                                                                                                                                                                                                           | 47                                                                                           | 32                                                                                           | 47                                                                                           | 47                                                                                           | 47                                                                                           | 47                                                                                           |
| Cover thickness (mm)                     |                                                                                                                                                                                                                                                                                                           | 1.5                                                                                          | 1.5                                                                                          | 1.5                                                                                          | 1.5                                                                                          | 1.5                                                                                          | 1.5                                                                                          |
| Ball                                     | Driver spin rate (rpm)<br>Driver flying distance (m)<br>Coefficient of restitution<br>Compression deformation amount (mm)                                                                                                                                                                                 | -90<br>4.0<br>0.017<br>3.74                                                                  | -20<br>2.5<br>0.011<br>3.84                                                                  | -30<br>2.0<br>0.010<br>3.71                                                                  | -60<br>2.3<br>0.009<br>3.96                                                                  | -110<br>2.6<br>0.006<br>3.89                                                                 | -80<br>2.8<br>0.007<br>3.63                                                                  |

TABLE 6

|                                          |                                      | Golf ball No. |       |       |       |        |       |      |
|------------------------------------------|--------------------------------------|---------------|-------|-------|-------|--------|-------|------|
|                                          |                                      | 20            | 21    | 22    | 23    | 24     | 25    | 26   |
| Rubber composition (parts by mass)       | BR730                                | 100           | 100   | 100   | 100   | 100    | 100   | 100  |
|                                          | Sanceler SR                          | 28            | 30    | 30    | 24    | 30     | 38    | 23   |
|                                          | Zinc oxide                           | 5             | 5     | 5     | 5     | 5      | 5     | 5    |
|                                          | Barium sulfate                       | *1)           | *1)   | *1)   | *1)   | *1)    | *1)   | *1)  |
|                                          | 2-Thionaphthol                       | 0.5           | 0.32  | 0.32  | 0.1   | 0.5    | 2     | —    |
|                                          | Stearic acid                         | —             | —     | —     | —     | —      | —     | —    |
|                                          | Zinc stearate                        | 10            | —     | —     | —     | —      | —     | —    |
|                                          | Myristic acid                        | —             | 10    | —     | —     | —      | —     | —    |
|                                          | Dicumyl peroxide                     | 0.8           | 0.8   | 0.8   | 0.8   | 0.8    | 0.8   | 0.8  |
|                                          | Total amount of carboxylic acid/salt | 12.8          | 13.0  | 3.0   | 2.4   | 3.0    | 3.8   | 2.3  |
| Core hardness distribution (JIS-C)       | Center hardness                      | 49.4          | 49.6  | 56.5  | 57.6  | 53.0   | 52.0  | 57.7 |
|                                          | 12.5% point hardness                 | 54.2          | 53.0  | 62.0  | 63.6  | 61.2   | 59.2  | 63.2 |
|                                          | 25% point hardness                   | 58.2          | 56.5  | 65.9  | 68.2  | 66.9   | 64.9  | 66.5 |
|                                          | 37.5% point hardness                 | 60.6          | 58.9  | 67.0  | 69.3  | 67.8   | 66.8  | 67.7 |
|                                          | 50% point hardness                   | 62.0          | 60.0  | 66.8  | 69.6  | 67.8   | 65.8  | 67.7 |
|                                          | 62.5% point hardness                 | 66.6          | 66.1  | 66.5  | 68.4  | 69.1   | 69.1  | 68.2 |
|                                          | 75% point hardness                   | 73.6          | 74.5  | 73.4  | 75.1  | 74.5   | 73.5  | 73.5 |
|                                          | 87.5% point hardness                 | 75.9          | 77.1  | 79.0  | 82.5  | 79.0   | 77.0  | 76.1 |
|                                          | Surface hardness                     | 80.7          | 81.0  | 84.1  | 86.9  | 82.7   | 80.7  | 81.4 |
|                                          | Surface hardness – center hardness   | 31.3          | 31.4  | 27.6  | 29.3  | 29.7   | 28.7  | 23.7 |
|                                          | R <sup>2</sup> of approximated curve | 0.98          | 0.97  | 0.89  | 0.89  | 0.92   | 0.94  | 0.92 |
|                                          | Slope of approximated curve          | 0.30          | 0.32  | 0.23  | 0.25  | 0.25   | 0.25  | 0.20 |
| Core coefficient of restitution          | 0.005                                | 0.012         | 0.012 | 0.007 | 0.004 | -0.001 | 0.000 |      |
| Core compression deformation amount (mm) | 4.39                                 | 4.12          | 4.06  | 4.00  | 4.17  | 4.33   | 4.29  |      |
| Cover composition                        | C                                    | C             | C     | C     | C     | C      | C     |      |
| Cover hardness (Shore D)                 | 47                                   | 47            | 47    | 47    | 47    | 47     | 47    |      |
| Cover thickness (mm)                     | 1.5                                  | 1.5           | 1.5   | 1.5   | 1.5   | 1.5    | 1.5   |      |
| Ball                                     | Driver spin rate (rpm)               | -90           | -70   | -10   | -20   | -30    | -30   | 0    |
|                                          | Driver flying distance (m)           | 2.0           | 2.7   | 0.7   | 0     | 0.5    | 0.3   | 0    |
|                                          | Coefficient of restitution           | 0.004         | 0.011 | 0.008 | 0.008 | 0.005  | 0     | 0    |
|                                          | Compression deformation amount (mm)  | 4.19          | 3.92  | 3.86  | 3.80  | 3.97   | 4.13  | 4.09 |

\*1) In tables No. 3 to 6, as to an amount of barium sulfate, adjustment was made such that the golf ball had a mass of 45.4 g.

BR730: a high-cis polybutadiene (cis-1,4 bond content = 96 mass %, 1,2-vinyl bond content = 1.3 mass %, Moony viscosity (ML<sub>1+4</sub> (100°C) = 55, molecular weight distribution (Mw/Mn) = 3) available from JSR Corporation

Sanceler SR: zinc acrylate (product of 10 mass % stearic acid coating) available from Sanshin Chemical Industry Co., Ltd.

Zinc oxide: "Ginrei R" manufactured by Toho Zinc Co., Ltd.

Barium sulfate: "Barium sulfate BD" manufactured by Sakai Chemical Industry Co., Ltd., adjustment was made such that the finally obtained golf ball had a mass of 45.4 g.

2-thionaphthol: manufactured by Tokyo Chemical Industry Co., Ltd.

Stearic acid: manufactured by NOF Corporation

Zinc stearate: manufactured by Wako Pure Chemical Industries, Ltd.

Myristic acid: manufactured by Tokyo Chemical Industry Co., Ltd. (Purity: 99.2%)

Dicumyl peroxide: "PERCUMYL ® D" manufactured by NOP Corporation

## (2) Production of Cover

Cover materials shown in Table 7 were mixed with a twin-screw kneading extruder to prepare the cover compositions in the pellet form. The extruding conditions of the cover composition were a screw diameter of 45 mm, a screw rotational speed of 200 rpm, and screw L/D=35, and the mixtures were heated to 150 to 230°C. at the die position of the extruder. The cover compositions obtained above were injection-molded onto the spherical cores to produce the golf balls having the spherical core and the cover covering the spherical core. The cover compositions having Shore D hardness of 50 or more were used for preparing distance-type golf balls No. 1 to No. 13 and the cover compositions having Shore D hardness of less than 50 were used to produce the spin-type golf balls No. 14 to No. 26.

TABLE 7

| Cover composition No. | A  | B  | C   | D   |
|-----------------------|----|----|-----|-----|
| Himilan 1605          | 50 | —  | —   | —   |
| Himilan 1706          | 50 | —  | —   | —   |
| Himilan 1855          | —  | 50 | —   | —   |
| Himilan 1856          | —  | 50 | —   | —   |
| Elastollan XNY97A     | —  | —  | 100 | —   |
| Elastollan XNY85A     | —  | —  | —   | 100 |

TABLE 7-continued

|    | Cover composition No.   | A  | B  | C  | D  |
|----|-------------------------|----|----|----|----|
| 45 | Titanium oxide          | 4  | 4  | 4  | 4  |
|    | Slab hardness (Shore D) | 65 | 55 | 47 | 32 |

Formulation: parts by mass

Himilan 1605: Sodium ion neutralized ethylene-methacrylic acid copolymer ionomer resin available from DuPont-Mitsui Polymers Co., Ltd

Himilan 1706: Zinc ion neutralized ethylene-methacrylic acid copolymer ionomer resin available from DuPont-Mitsui Polymers Co., Ltd

Himilan 1855: Zinc ion neutralized ethylene-methacrylic acid-isobutylacrylate copolymer ionomer resin available from DuPont-Mitsui Polymers Co., Ltd

Himilan 1856: Sodium ion neutralized ethylene-methacrylic acid-isobutylacrylate copolymer ionomer resin available from DuPont-Mitsui Polymers Co., Ltd

Elastollan XNY85A: Thermoplastic polyurethane elastomer available from BASF Japan Co.

Elastollan XNY97A: Thermoplastic polyurethane elastomer available from BASF Japan Co.

From the evaluation of Tables 3 to 6, it is clear that the golf ball comprising a spherical core and at least one cover layer covering the spherical core, wherein the spherical core of the golf ball is formed from the rubber composition comprising (a) the base rubber, (b) the co-crosslinking agent, (c) the crosslinking initiator, (d) the carboxylic acid and/or the salt thereof, and (e) the organic sulfur compound having the naphthalene ring, provided that the rubber composition further contains (f) a metal compound in the case of containing only (b) the  $\alpha,\alpha$ -unsaturated carboxylic acid having 3 to 8 carbon atoms as the co-crosslinking agent has a low spin rate and travels a great flight distance on driver shots.

The golf ball of the present invention travels a great flight distance on the driver shots. This application is based on Japanese Patent applications No. 2010-294591 filed on Dec. 29, 2010.

The invention claimed is:

1. A golf ball having a spherical core and at least one cover layer covering the spherical core, wherein the spherical core is formed from a rubber composition containing:

(a) a base rubber,  
(b) an  $\alpha,\beta$ -unsaturated carboxylic acid having 3 to 8 carbon atoms and/or a metal salt thereof as a co-crosslinking agent,

(c) a crosslinking initiator,  
(d) a carboxylic acid and/or a carboxylic acid salt, and  
(e) an organic sulfur compound having a naphthalene ring, provided that the rubber composition further contains (f) a metal compound in the case of containing only (b) the  $\alpha,\beta$ -unsaturated carboxylic acid having 3 to 8 carbon atoms as the co-crosslinking agent;

wherein the rubber composition contains (d) the carboxylic acid and/or the carboxylic acid salt in an amount ranging from 7.5 parts to 40 parts by mass with respect to 100 parts by mass of (a) the base rubber;

wherein the carboxylic acid salt includes zinc laurate, zinc myristate, zinc palmitate, zinc stearate, zinc behenate, zinc montanate, or zinc 12-hydroxystearate, and wherein if the JIS-C hardness is measured in the spherical core at nine points obtained by dividing the radius of the spherical core into equal parts having 12.5% interval therebetween, and is plotted on a graph against distance (%) from the spherical core center, the  $R^2$  value of a linear approximation curve obtained from the least square method is 0.95 or higher.

2. The golf ball according to claim 1, wherein the rubber composition contains (d) the carboxylic acid in an amount ranging from 7.5 parts by mass to 20 parts by mass with respect to 100 parts by mass of (a) the base rubber.

3. The golf ball according to claim 1, wherein the rubber composition contains (d) the carboxylic acid salt in an amount ranging from 10 parts by mass to 25 parts by mass with respect to 100 parts by mass of (a) the base rubber.

4. The golf ball according to claim 1, wherein the rubber composition contains (e) the organic sulfur compound having the naphthalene ring in an amount ranging from 0.05 part to 5 parts by mass with respect to 100 parts by mass of (a) the base rubber.

5. The golf ball according to claim 1, wherein (e) the organic sulfur compound having the naphthalene ring includes thionaphthol or a derivative thereof.

6. The golf ball according to claim 5, wherein the rubber composition contains thionaphthol or a derivative thereof in an amount ranging from 0.05 part to 2 parts by mass with respect to 100 parts by mass of (a) the base rubber.

7. The golf ball according to claim 1, wherein the rubber composition contains (b) the metal salt of the  $\alpha,\beta$ -unsaturated carboxylic acid having 3 to 8 carbon atoms as the co-crosslinking agent.

8. The golf ball according to claim 1, wherein (d) the carboxylic acid is a fatty acid.

9. The golf ball according to claim 1, wherein (d) the carboxylic acid is a carboxylic acid having 4 to 30 carbon atoms.

10. The golf ball according to claim 1, wherein (d) the carboxylic acid is a carboxylic acid having 9 to 30 carbon atoms.

11. The golf ball according to claim 1, wherein the rubber composition contains (b) the  $\alpha,\beta$ -unsaturated carboxylic acid having 3 to 8 carbon atoms and/or the metal salt thereof in an amount ranging from 15 parts by mass to 50 parts by mass with respect to 100 parts by mass of (a) the base rubber.

12. A golf ball having a spherical core and at least one cover layer covering the spherical core, wherein the spherical core is formed from a rubber composition containing:

(a) a base rubber,  
(b) an  $\alpha,\beta$ -unsaturated carboxylic acid having 3 to 8 carbon atoms and/or a metal salt thereof as a co-crosslinking agent,

(c) a crosslinking initiator,  
(d) a carboxylic acid having 4 to 10 carbon atoms and/or a salt thereof, and  
(e) thionaphthol or a derivative thereof,

provided that the rubber composition further contains (f) a metal compound in the case of containing only (b) the  $\alpha,\beta$ -unsaturated carboxylic acid having 3 to 8 carbon atoms as the co-crosslinking agent, and

wherein if the JIS-C hardness is measured in the spherical core at nine points obtained by dividing the radius of the spherical core into equal parts having 12.5% interval therebetween, and is plotted on a graph against distance (%) from the spherical core center, the  $R^2$  value of a linear approximation curve obtained from the least square method is 0.95 or higher.

13. The golf ball according to claim 12, wherein the rubber composition contains thionaphthol or the derivative thereof in an amount ranging from 0.05 part to 2 parts by mass with respect to 100 parts by mass of (a) the base rubber.

14. The golf ball according to claim 12, wherein the rubber composition contains (d) the carboxylic acid having 4 to 10 carbon atoms and/or the salt thereof in an amount ranging from 5 parts to 40 parts by mass with respect to 100 parts by mass of (a) the base rubber.

15. The golf ball according to claim 12, wherein the rubber composition contains (d) the carboxylic acid having 4 to 10 carbon atoms in an amount ranging from 5 parts by mass to 20 parts by mass with respect to 100 parts by mass of (a) the base rubber.

16. The golf ball according to claim 12, wherein the rubber composition contains (d) the salt of the carboxylic acid having 4 to 10 carbon atoms in an amount ranging from 10 parts by mass to 25 parts by mass with respect to 100 parts by mass of (a) the base rubber.

17. The golf ball according to claim 12, wherein the spherical core has a hardness difference of 15 or more in JIS-C hardness between a surface hardness and a center hardness thereof.

18. The golf ball according to claim 12, wherein the rubber composition contains (b) the metal salt of the  $\alpha,\beta$ -unsaturated carboxylic acid having 3 to 8 carbon atoms as the co-crosslinking agent.

19. The golf ball according to claim 12, wherein (d) the carboxylic acid and/or the salt thereof is a fatty acid and/or a fatty acid salt.